# EUROPEAN PATENT SPECIFICATION

(11) **EP 0 745 180 B1**
(45) Date of publication and mention of the grant of the patent: **03.04.2002**
(21) Application number: 95911772.2
(22) Date of filing: 28.02.1995
(51) Int. Cl.: F01N 3/28, F23C 11/00, B01J 35/04

(54) **IMPROVED PROCESS AND CATALYST STRUCTURE EMPLOYING INTEGRAL HEAT EXCHANGE WITH OPTIONAL DOWNSTREAM FLAMEHOLDER**
VERBESSERTE VERFAHREN UND KATALYTISCHE, STRUKTUR, BENUTZEND INTEGRALEN WÄRMEAUSTAUSCH MIT WAHLWEISE VORGESCHALTETEM FLAMMENHALTER
PROCEDE ET STRUCTURE CATALYTIQUES AMELIORES ASSURANT UN ECHANGE THERMIQUE INTEGRAL AVEC EVENTUELLEMENT UNE FLAMME ENTRETENUE EN AVAL

(30) Priority: 02.03.1994 US 205279; 25.01.1995 US 378206
(43) Date of publication of application: 04.12.1996
(73) Proprietor: CATALYTICA, INC., Mountain View, CA 94043-5272 (US); TANAKA KIKINZOKU KOGYO K.K., Chuo-ku Tokyo 103 (JP)
(72) Inventor: DALLA BETTA, Ralph, A., Mountain View, CA 94040 (US); SHOJI, Toru, Hiratsuka-city Kanagawa (JP); YEE, David, K., Hayward, CA 94544 (US); MAGNO, Scott, A., Dublin, CA 94568 (US)
(74) Representative: Price, Nigel John King
(86) International application number: US9501989
(87) International publication number: WO9523915

(56) References cited:
- DE-A- 4 202 108
- DE-C- 4 202 018
- US-A- 3 568 462
- US-A- 4 731 989
- US-A- 4 870 824
- US-A- 4 936 380
- US-A- 5 183 401
- US-A- 5 202 303

## Description

### FIELD OF THE INVENTION

This invention relates to a catalyst structure employing integral heat exchange in an array of longitudinally disposed, adjacent reaction passageways or channels which are either catalyst-coated or catalyst-free, as well as a method for using the catalyst structure in highly exothermic processes, such as combustion or partial combustion processes. More particularly, this invention is directed to such a catalyst structure employing integral heat exchange wherein the catalytic and non-catalytic channels differ from each other in certain critical respects whereby the exothermic reaction in the catalytic channels and heat exchange between the catalytic and non-catalytic channels are optimized while undesired exothermic reaction in the non-catalytic channels is suppressed.

### BACKGROUND OF THE INVENTION

In modem industrial practice, a variety of highly exothermic reactions are known to be promoted by contacting of the reaction mixture in the gaseous or vapor phase with a heterogeneous catalyst. In some cases these exothermic reactions are carried out in catalyst-containing structures or vessels where external cooling must be supplied, in part, because of the inability to obtain sufficient heat transfer and the need to control the reaction within certain temperature constraints. In these cases, it is not considered practical to use a monolithic catalyst structure, where the unreacted portion of the reaction mixture supplies the cooling for the catalytic reaction, because existing catalyst structures do not provide an environment whereby the desired reaction can be optimized while removing the heat of reaction through heat exchange with unreacted reaction mixture under conditions where undesired reactions and catalyst overheating are avoided. Thus, the applicability of monolithic catalysts structures to many catalyzed exothermic reactions could clearly be enhanced if monolithic catalyst structures could be developed wherein the reaction zone environment and heat exchange between reacted and unreacted portions of the reaction mixture are improved.

There is also a clear need to improve the operability of monolithic catalyst structures in areas where they are currently used or proposed for use, such as the combustion or partial combustion of fuels or the catalytic treatment of exhaust emissions from internal combustion engines, to widen the range of operating, conditions at which the desired catalytic conversions can be achieved. For example, in the case of catalytic combustion when applied to reduce NOₓ emissions from a gas turbine by equipping the turbine with a catalytic combustor, a clear need exists for catalytic systems or structures which will adapt to a variety of operational situations. A gas turbine used as a power source to drive a load must be operated over a range of speeds and loads to adjust power output to the load requirements. This means that the combustor must operate over a range of air and fuel flows. If the combustor system uses a catalyst to combust the fuel and limit emissions, then this catalyst system must be able to operate over a wide range of air flows, fuel/air ratios (F/A) and pressures.

Specifically in the case of an electric power generation turbine where the rotational speed is constant because of the need to generate power at a constant frequency, the air flow over the load range of 0% to 100% will be approximately constant. However, the fuel flow will vary to match the load required so the F/A will vary. In addition, the pressure will increase somewhat as the power output is increased. This means that the catalytic combustor must operate over a wide range of F/A and a range of pressures but at relatively constant mass flow. Alternatively, a variable portion of the air flow can be bypassed around the combustor or bled from the gas turbine to decrease the air flow and maintain a more constant F/A. This will result in a narrower range of F/A over the catalyst but a wider range of mass flows.

Further, in the case of a variable speed turbine, or a multiple shaft turbine, the air flow and pressure can vary widely over the operating range. This results in a wide variation of total mass flow and pressure in the combustor. Similar to the situation described above for the electric power generation turbine, the air can be bypassed or bled to control the F/A range resulting in a combustor that must operate over a range of mass flows.

The situations described above result in the need for a catalyst design that can operate over a wide mass flow range, pressure range and F/A range.

One particular application that could benefit from catalytic combustion is a gas turbine applied to a vehicle to achieve very low emissions. Once started, this engine must operate from idle to full load and achieve low emissions over this entire range. Even if the gas turbine is used in a hybrid vehicle design combined with a storage component such as a battery, flywheel, etc., the engine must still operate at idle and full load and must transit between these two operating points. This requires operation at mass flows and pressures of both of these conditions.

The present invention employs a catalyst structure made up of a series of adjacently disposed catalyst-coated and catalyst-free channels for passage of a flowing reaction mixture, wherein the catalytic and non-catalytic channels share a common wall such that integral heat exchange can be used to dissipate the reaction heat generated on the catalyst and thereby control or limit the temperature of the catalyst. That is, the heat produced on the catalyst in any given catalyst-coated channel flows through the common wall to the opposite non-catalytic surface to be dissipated into the flowing reaction mixture in the adjacent catalyst-free channel. With the present invention, the configuration of the catalytic channels differs from the non-catalytic channels in one or more critical respects, in particular the tortuosity of the flow channel, such that, when applied to catalytic combustion, catalytic and homogeneous combustion is promoted within the catalytic channels and not promoted or substantially limited in the non-catalytic channels while heat exchange is otherwise optimized. These uniquely configured catalyst structures substantially widen the window of operating parameters for catalytic combustion and/or partial combustion processes.

The use of catalyst supports having integral heat exchange in catalyst-promoted combustion or partial combustion is known in the art. In particular, Japanese Kokai 59-136,140 (published August 4, 1984) and Kokai 61-259,013 (published November 17, 1986) disclose the use of integral heat exchange in either a square-sectioned ceramic monolithic catalyst support in which alternating longitudinal channels (or layers) have catalysts deposited therein, or a support structure made up of concentric cylinders in which alternating annular spaces in the support are coated with catalyst. In both cases, the design of the catalyst structure disclosed is such that the configuration of the catalyst-coated channels and catalyst-free channels is the same with the catalytic and non-catalytic flow channels in each case being essentially straight and of the same cross-sectional area throughout their lengths.

A disclosure very similar to the two Japanese Kokai is seen in U.S. Patent No. 4,870,824 to Young et al. where integral heat exchange is employed is a honeycomb support structure in which the catalyst-coated and catalyst-free channels are of identical configuration, being essentially straight and of unvarying square cross-sectional area throughout their length.

US 5,202,303 discloses a multiple-stage combustion apparatus which can be used in a high-temperature environment, such as with a gas turbine. A first stage, which is an ignition stage, is a reactor formed of a metal strip which is coated with a catalyst on only one side. The strip is also corrugated with a herringbone pattern. The strip is then folded back and forth upon itself to form a reactor of a desired cross-section. The reactor has rows of channels that are formed between the layers of the metal. The single coated side of the metal defines the walls of the channels in every other row. The fuel-air mixture that flows through the coated channels is combusted. The one or more stages subsequent to the ignition stage can employ a catalyst capable of operating at the very high temperatures present in gas turbines. The subsequent stages can also be non-catalytic. Thus, the first stage provides catalytic ignition, and the subsequent stages complete the combustion.

DE 4202018 C1 discloses a method for stabilising a catalytically supported combustion. A flame holder is located downstreams a catalyst. Thereby a recirculation zone is established which results in a stable after-burning in a consecutive homogeneous combustion zone.

More recently, a series of U.S. patents have issued to Dalla Betta et al., including U.S. Patent Nos. 5,183,401; 5,232,357; 5,248,251; 5,250,489 and 5,259,754, which describe the use of integral heat exchange in a variety of combustion or partial combustion processes or systems, including those where partial combustion of the fuel occurs in aN integral heat exchange structure followed by subsequent complete combustion after the catalyst. Of these U.S. patents, U.S. Patent No. 5,250,489 seems most in point, being directed to a metallic catalyst support made up of a high temperature resistant metal formed into a multitude of longitudinal passageways for passage of a combustible gas, with integral heat exchange being employed between passageways at least partially coated with catalyst and catalyst-free passageways to remove heat from the catalytic surface in the catalyst-coated passageways. The catalytic support structures disclosed in this patent include structures (FIGS. 6A and 6B) wherein the combustible gas passageways or channels are formed by alternating broad or narrow corrugations of a corrugated metal foil such that the size of the alternating catalytic and non-catalytic channels are varied to allow 80% of the gas flow to pass through the catalytic channels and 20% through the non-catalytic channels in one case (FIG. 6A), or 20% of the gas flow to pass through the catalytic channels and 80% through the non-catalytic channels in the other case (FIG. 6B). Using different sized channels as a design criterion, this patent teaches that any level of combustible gas conversion to combustion products between 5% and 95% can be achieved while incorporating integral heat exchange. While this patent does disclose the use of different sized catalytic and non-catalytic channels to vary the level of conversion, it clearly does not contemplate the use of channels having different tortuosity in the catalytic versus non-catalytic channels to optimize the combustion reaction in catalytic channels while substantially limiting homogeneous combustion in the non-catalytic channels as a means of widening the range of process conditions under which the catalyst structure can effectively operate.

In cases where the integral heat exchange structure is used to carry out catalytic partial combustion of a fuel followed by complete combustion after the catalyst, the catalyst must burn a portion of the fuel and produce an outlet gas sufficiently hot to induce homogeneous combustion after the catalyst. In addition, it is desirable that the catalyst not become too hot since this would shorten the life of the catalyst and limit the advantages to be gained from this approach. As the operating condition of the catalyst is changed, it is noted with the integral heat exchange structures of the prior art, discussed above, that operating window of such catalysts are limited. That is, that the gas velocity or mass flow rate must be within a certain range to prevent catalyst overheating.

Therefore, it is clear that a need exists for improved catalytic structures employing integral heat exchange which will substantially widen the window or range of operating conditions under which such catalytic structures can be employed in highly exothermic processes like catalytic combustion or partial combustion. The present invention capitalizes on certain critical differences in the configuration of the catalytic and non-catalytic passageways or channels in an integral heat exchange structure to materially widen the operating window for such catalysts.

According to the present invention, a reaction system for a combustion of a combustible mixture of fuel as defined in independent claims 1 and 8, and a process for combustion of a combustible mixture, as defined in independent claims 17 and 18, is proposed.

In particular, it may be provided a catalyst structure comprised of a series of adjacently disposed catalyst-coated and catalyst-free channels for passage of a flowing reaction mixture wherein the channels at least partially coated with catalyst are in heat exchange relationship with adjacent catalyst-free channels and wherein the catalyst-coated channels have a configuration which forms a more tortuous flow passage for the reaction mixture than the flow passage formed by the catalyst-free channels. For convenience herein the terms "catalyst-coated channels" or "catalytic channels" in the catalyst structures of the invention may refer to single channels or groupings of adjacent channels which are all coated with catalyst on at least a portion of their surface, in effect a larger catalytic channel subdivided into a series of smaller channels by catalyst support walls or pervious or impervious barriers which may or may not be coated with catalyst. Similarly, the "catalyst-free channels" or "non-catalytic channels" may be a single channel or grouping of adjacent channels which are all not coated with catalyst, that is, a larger catalyst-free channel subdivided into a series of smaller channels by catalyst support walls or pervious or impervious barriers which are not coated with catalyst. In this regard, increased tortuosity of the flow passages formed by the catalyst-coated channels means that the catalyst-coated channels are designed such that at least a portion of the reaction mixture entering the catalyst-coated channels will undergo more changes in direction of flow as it traverses the length of the channel than will any similar portion of reaction mixture entering the catalyst-free channels. Ideally, if it were assumed that the longitudinal axes of the catalyst-coated channels is a straight line leading from the inlet of the channel to the outlet of the channel, increasing the tortuosity of the channel would result in a reaction mixture flow pathway which shows increasing directional deviations from the axis such that the path traveled by tracing the deviations becomes increasing longer than the path drawn by the axis.

In practice, the increased tortuosity of the flow passage in the catalyst-coated channels can be accomplished by a variety of structural modifications to the channels including periodically altering their direction and/or changing their cross-sectional area along their longitudinal axis while the catalyst-free channels remain substantially straight and unaltered in cross-sectional area. Preferably the tortuosity of the catalyst-coated channels is increased by varying their cross-sectional area though repeated inward and outward bending of channels walls along the longitudinal axis of the channels or through the insertion of flaps, baffles or other obstructions at a plurality of points along the longitudinal axes of the channels to partially obstruct and/or divert the direction of reaction mixture flow in the channels.

In a preferred aspect, the catalyst structure can be further characterized by catalyst-coated channels that differ from the catalyst-free channels in one or more critical structural defining elements which, in turn, take advantage of, and expand upon, the concept of the increased tortuosity of the catalyst-coated channels. In particular, the preferred catalyst structure of the invention typically employs a plurality of longitudinally disposed channels coated on at least a portion of their interior surface with catalyst, that is, catalyst-coated channels, in heat exchange relationship with adjacent channels not coated with catalyst or catalyst-free channels wherein:
(a) the catalyst-coated channels have an average hydraulic diameter (Dₕ) which is lower than the average hydraulic diameter of the catalyst-free channels and/or;
(b) the catalyst-coated channels have a higher film heat transfer coefficient (h) than the catalyst-free channels.

The average hydraulic diameter or Dₕ, which is defined as four times the average cross-sectional area of ail of the channels of a particular type, e.g., catalyst-coated channels, in the catalyst structure divided by the average wetted perimeter of all of the channels of that type in the catalyst structure, is reflective of the finding that the catalyst-free channels are most advantageously designed to have a larger hydraulic diameter and to be less effected by changes in configuration than the catalyst-coated channels. The film heat transfer coefficient or h is an experimentally determined value which correlates with, and expands upon the tortuosity of the average catalyst-coated channel versus that of the average catalyst-free channel in the catalyst structure.

Further optimization of the catalyst structure is obtained if, in addition to controlling the average Dₕ and/or h as set forth above, the heat transfer surface area between the catalyst-coated channels and the catalyst-free channels is controlled such that the heat transfer surface area between the catalyst-coated channels and catalyst-free channels divided by the total channel volume in the catalyst structure is greater than about 0.5 mm⁻¹.

The catalyst structure is particularly useful when equipped with appropriate catalytic materials for use in a combustion or partial combustion process wherein a fuel, in gaseous or vaporous form, is typically partially combusted in the catalyst structure followed by complete homogeneous conibustion downstream of the catalyst With the catalyst structure, it is possible to obtain more complete combustion of fuel in the catalytic channels with minimum combustion in the non-catalytic channels over a wider range of linear velocities, gas inlet temperatures and pressures than has here-to-for been possible with catalyst structures of the prior art, including those employing integral heat exchange. Accordingly, the invention also encompasses a catalyst structure for use in the combustion or partial combustion of a combustible fuel, as well as a process for combusting a mixture of a combustible fuel and air or oxygen-containing gas, using the catalyst structure.

In an additional aspect which is applicable to combustion or partial combustion processes employing integral heat exchange type-catalyst structures, including the catalyst structures, involves the addition of a flameholder or other means for inducing recirculation into the partially combustible gas mixture flowing into a homogeneous combustion zone immediately downstream from the outlet end of the catalyst structure. The addition of a flameholder or other means for inducing gas recirculation downstream of the outlet end of the catalyst structure provides additional flexibility in the range of suitable operating parameters for catalytic combustion and/or partial combustion processes, including reduced catalyst operating temperatures which could have an overall favorable effect on catalyst lifetimes.

### BRIEF DESCRIPTION OF THE DRAWINGS

FIGS. 1, 2, 3, 3A, 3B, and 3C schematically depict configurations of the prior art showing conventional forms of catalytic structures employing integral heat exchange.
FIGS. 4, 5, 6, 7, and 8 show various configurations of the inventive catalyst structure.
FIGS. 9 and 10 are schematic representations of a reaction system according to the invention where a flameholder is positioned at the outlet end of the catalyst structure in the homogeneous combustion zone.
FIGS. 11A through 14B show several different configurations of flameholders which may be employed in the homogeneous combustion zone downstream of the catalyst structure in accordance with the invention.
FIGS. 15 and 16 show the effects of a flameholder on the temperature of the combustion gas downstream of a catalyst structure according to the invention versus Tad of the fuel/air inlet mixture.

### DETAILED DESCRIPTION

When applied to the catalysis of highly exothermic reactions, the catalyst structures of the invention are typically monolithic-type structures comprising a heat resistant support material composed of a plurality of common walls which form a multitude of adjacently disposed longitudinal channels for passage of a gaseous reaction mixture wherein at least a portion of the channels are coated on at least a part of their interior surface with a catalyst for the reaction mixture (catalyst-coated channels) and the remaining channels are not coated with catalyst on their interior surface (catalyst-free channels) such that the interior surface of the catalyst-coated channels are in heat exchange relationship with the interior surface of adjacent catalyst-free channels and wherein the catalyst-coated channels differ in configuration from the catalyst-free channels such that the desired reaction is promoted in the catalytic channels and suppressed in the non-catalytic channels. In cases where the catalyst structure of the invention is employed in a catalytic combustion or partial combustion process, the critical difference in the design of the catalytic versus non-catalytic channels will insure more complete combustion of the fuel in the catalytic channels and minimum combustion in the non-catalytic channels over a wider range of linear velocity, inlet gas temperature and pressure.

The critical difference in the design of the catalytic versus non-catalytic channels for the catalytic structure of the invention, in its most basic terms, is that the catalytic channels are designed so that the reaction mixture flow passages defined by the catalytic channels possess a higher or increased tortuosity over the corresponding flow passages formed by the non-catalytic channels. The concept of tortuosity, as used herein, is defined as the difference between the length of the path which a given portion of reaction mixture will travel through the passage formed by the channel as a result of changes in direction of the channel and/or changes in channel cross-sectional area versus the length of the path traveled by a similar portion of the reaction mixture in a channel of the same overall length without changes in direction or cross-sectional area, in other words, a straight channel of unaltered cross-sectional area. The deviations from a straight or linear path, of course, result in a longer or more tortuous path and the greater the deviations from a linear path the longer the traveled path will be. When applied to the catalyst structures of the invention, differences in tortuosity between catalytic and non-catalytic channels is determined by comparing the average tortuosity of all of the catalytic channels in the structure to the average tortuosity of all of the non-catalytic channels in the structures.

In the catalyst structures of the invention a variety of structure modifications can be made to the channels coated with catalyst to increase their tortuosity relative to the non-catalytic channels. In particular, the tortuosity of the catalytic channels can be increased by periodically changing their direction, for example, by using channels having a zig-zag or wavy configuration or by repeatedly changing their cross-sectional area through periodic inward and outward bending of channel walls along their longitudinal axis or through the insertion of flaps, baffles or other obstructions to partially obstruct or divert the direction of reaction mixture flow at a plurality of points along the longitudinal axis of the channel. In some applications, it may be desirable to use a combination of changes in direction and changes in cross-sectional area to achieve an optimum difference in tortuosity but in all cases the tortuosity of the non-catalytic channel will be less on average than the tortuosity of the catalytic channels.

Preferably, the tortuosity of the catalytic channels is increased by changing their cross-sectional area at a multiplicity of points along their longitudinal axes. One preferred way of accomplishing this change in tortuosity for the catalytic channels, which is discussed in further detail below, involves the use of a stacked arrangement of non-nesting corrugated sheets of catalyst support material which are corrugated in a herringbone pattern with at least a portion of one side of a given corrugated sheet facing and stacked against another corrugated sheet being coated with catalyst such that the stacked sheets in question form a plurality of catalytic channels. By stacking the corrugated sheets together in a non-nesting fashion, the channels formed by the stacked sheets alternately expand and contract in cross-sectional area along their longitudinal axis due to the inwardly and outwardly bending peaks and valleys formed by the herringbone pattern of the corrugated sheets. Other preferred ways of changing the cross-sectional area of the catalyst-coated channels include the periodic placement of flaps or baffles on alternate sides of the channels along their longitudinal axis or the use of screens or other partial obstructions in the flow path formed by the catalytic channels. To avoid undue pressure drops across the channel the cross-sectional area of the channel should not be reduced by more than about 40% of its total cross-sectional area by any obstruction placed in the flow path formed by the channel.

As noted previously, in preferred catalyst structures of the invention the channels coated with catalyst differ from the catalyst-free channels by having an average hydraulic diameter (Dₕ) which is lower than the average hydraulic diameter of the catalyst-free channels and/or by having a higher film heat transfer coefficient (h) than the catalyst-free channels. More preferably, the catalyst-coated channels have both a lower Dₕ and a higher h than the catalyst-free channels.

The average hydraulic diameter is defined in Whitaker, *Fundamental Principles of Heat Transfer,* Krieger Publishing Company (1983) at page 296 by the following formula: Thus, for the catalyst structures of the invention, the average Dₕ can be determined by first finding the Dₕ for all of the catalyst-coated channels in the structure by calculating the average Dₕ for any given channel over its entire length and then determining the average Dₕ for the catalyst-coated channels by totalling up all of the calculated Dₕs for the individual channels, multiplied by a weighing factor representing the fractional open frontal area for that channel. Following the same procedure, the average Dₕ for the catalyst-free channels in the structure can also be determined.

As discussed above, the finding that the catalyst-coated channels most advantageously have a lower average Dₕ than the catalyst-free channels can be explained, in part, by the fact that the catalyst-coated channels desirably have a surface to volume ratio which is higher than that of the catalyst-free channels, since hydraulic diameter bears an inverse relationship to surface to volume ratio. Further, in the catalyst structures of the invention, the difference in average Dₕ of the catalyst-coated channels and catalyst-free channels gives an indication that the catalyst-free channels, on average, must be more open channeled and therefore, the gas flow through these channels is less effected by changes in the channel diameter than the catalyst-coated channels, again, in part, because of the higher surface to volume ratios in the catalyst-coated channels. Preferably, the numeric ratio of the average Dₕ of the catalyst-coated channels to the average Dₕ of the catalyst-free channels, that is, average Dₕ of catalyst-coated channels divided by average Dₕ of catalyst-free channels is between about 0.15 and about 0.9 and, most preferably, the ratio of average Dₕ of catalyst-coated channels to catalyst-free channels is between about 0.3 and 0.8.

The film heat transfer coefficient (h) is a dimension-less value, which is measured experimentally by flowing gas, e.g., air or air/fuel mixtures, at a given inlet temperature through an appropriate test structure having the specified channel geometry and temperature and measuring the outlet gas temperature, with h being calculated using the experimentally determined values in the following equation which describes heat transfer for an incremental portion of the flow path Δx (adapted from Whitaker, *Ibid.*, equations 1.3-29 and 1.3-31 on pages 13 and 14):${\text{FC}}_{\text{p}} \text{(ΔTgas) = h A (Twall-Tgas) Δx}$ where
F is the gas flow rate;
Cₚ is the heat capacity of the gas;
h is the heat transfer coefficient;
A is the wall area per unit channel length;
ΔTgas is the temperature rise in the gas stream over the incremental distance Δx;
Twall is the wall temperature at position x; and
T gas is the gas temperature at position x.
Integration of this equation from the inlet to the outlet of the test structure will allow determining the value of film heat transfer coefficient that gives a calculated outlet gas temperature that matches experiment.

Since the gas composition, flow rates, pressures and temperatures in the catalytic and non-catalytic channels of the catalyst structure of the invention are very similar, the film heat transfer coefficient provides useful means of characterizing the different flow geometries provided by the various flow channel configurations which distinguish the catalyst-coated channels from the catalyst-free channels of the catalyst structure according to the invention.

Since these different flow geometries, in turn, are related to the tortuosity of the flow path formed by the channels, the film heat transfer coefficient provides some measure of tortuosity as it is employed in the catalyst structures of the invention. While one skilled in the art could conceive of a variety of methods to measure or otherwise determine h in the catalyst structures of the invention, one convenient method would involve constructing an experimental test structure, for example, a solid thick metal structure, with internal space machined to simulate the desired channel shape; and then to test it in environments where the wall temperature is essentially constant from inlet to outlet or varies from inlet to outlet and is measured at several points along the channel length in the structure. For monoliths such as the straight channel structure depicted in FIG. 1 (see discussion below), the test structure can be a single channel or a linear array of channels. For a herringbone corrugation monolith such as that shown in FIG. 2 (also discussed below), the test structure would be a section of the linear region containing channels of non-nesting herringbone configuration between two metal sheets sufficiently wide to minimize side effects.

The above-described technique can be applied to any of the structures described herein by constructing the required test structure. In cases where the catalyst structure is a combination of several different channel configurations, each of the channel configurations can be tested separately and the numeric ratio for h(cat)/h(non-cat) can be determined by summing up the h's for each channel type (multiplied by a weighing factor representing the fractional open frontal area) in the catalyst structure and then dividing the sum of the h's for the catalytic channels by the sum of the h's for the non-catalytic channels.

The h(cat)/h(non-cat) ratios which characterize the difference in the configuration of the catalyst-coated and catalyst-free channels in the catalyst structure of the invention are further defined by the principle that in cases where h(cat)/h(non-cat) is greater than 1, the numeric ratio of the average hydraulic diameter (Dₕ) for the catalyst-coated channels divided by the average Dₕ for the catalyst-free channels is smaller than the numeric ratio of the open frontal area of the catalyst-coated channels divided by the open frontal area of the catalyst-free channels. As used herein, open frontal area refers to the cross-sectional area of channels of a given type, i.e., catalytic or non-catalytic, averaged over the catalyst structure in question; the cross-sectional area being the area open to reaction mixture flow in a channel, measured perpendicular to the reaction mixture flow direction. Introduction of this numeric ratio based on open frontal area is reflective of the fact that the catalyst-coated channels of the present invention have a sufficient increase in tortuosity over the catalyst-free channels to be clearly distinguishable from prior art structures employing integral heat exchange where the flow ratio through catalytic and non-catalytic channels is controlled by the use of different sized channels of the same basic configuration. That is, in cases where the reaction mixture flow is less than 50% through the catalytic channels in such prior art structures, the catalytic channels have a smaller average Dₕ than the non-catalytic channels and the ratio of h(cat)/h(non-cat) can exceed 1. By introducing the concept that the numeric ratio of average Dₕ for catalytic channels divided by average Dₕ for non-catalytic channels must be smaller than the numeric ratio of open frontal area for catalytic channels divided by open frontal area of non-catalytic channels the catalyst structures of the present invention can be clearly differentiated from the prior art structures.

Alternatively, the catalyst structures of the present invention can be distinguished by the use of higher film heat transfer coefficients (h) for the catalytic channels verses non-catalytic channels than is characteristic of the prior art structures employing catalytic and non-catalytic channels which are of different size but the same basic configuration. In a prior art straight channel structure with catalytic channels that represent 20% of the open frontal area and non-catalytic channels representing 80% of the open frontal area, the heat transfer coefficient of the catalytic channels would be approximately 1.5 times the heat transfer coefficient of the non-catalytic channels. The structures of this invention would have heat transfer coefficients in the catalytic channels substantially larger than 1.5 times the heat transfer coefficient of the non-catalytic channels. More specifically, for catalyst structures having various reaction flow distributions between catalytic and non-catalytic channels, the following table defines catalyst structures of the invention.

| Percent of Total Reaction Mixture Flow through Catalytic Channels | Ratio of h(cat)/h(non-cat) |
|---|---|
| 50 and higher | >1.0 |
| Less than 50 but more than 40 | >1.2 |
| Less than 40 but more than 30 | >1.3 |
| Less than 30 but more than 20 | >1.5 |
| Less than 20 but more than 10 | >2.0 |

In any case, if the ratio of h(cat)/h(non-cat) is greater than 1, that is, h for the catalyst-coated channels is higher than h for the catalyst-free channels, then the catalyst structure is within the scope of the present invention. Preferably, catalyst structures of the invention have h(cat)/h(non-cat) ratios in the range of about 1.1 and about 7, and most preferably the ratio is between about 1.3 and about 4.

As noted previously, the performance of the catalyst structures of the invention can be further optimized if the catalyst-coated and catalyst-free channels are configured such that the heat transfer surface area between the catalyst-coated and the catalyst-free channels divided by the total channel volume in the catalyst structure is greater than about 0.5 mm⁻¹. In preferred catalyst structures of the invention, the ratio of heat transfer area between the catalyst-coated and the catalyst-free channels divided by the total channel volume in the catalyst structure or R is between about 0.5 mm⁻¹ and 2 mm⁻¹ with Rs in the range of about 0.5 mm⁻¹ to about 1.5 mm⁻¹ being most preferred. With these high heat transfer surface to total volume ratios or Rs, the transfer of heat from the catalyst to the non-catalytic side of the channel wall for dissipation into the flowing reaction mixture is optimized. With optimum removal of heat from the catalytic surface by this integral heat exchange, it is possible to operate the catalyst under more severe conditions without causing overheating of the catalyst. This is advantageous since it contributes to widening the range of conditions under which the catalyst can be operated.

The catalyst structures of the invention can be designed to operate over a wide reaction mixture flow distribution between the catalytic and non-catalytic channels. By controlling the size and number of catalytic versus non-catalytic channels in the catalyst structure between about 10% and about 90% of the total flow can be directed through the catalytic channels depending on the exothermic nature of the reaction being catalyzed and the extent of conversion desired. Preferably, in highly exothermic processes like combustion or partial combustion of a fuel, the ratio of reaction mixture flow through the catalyst structure is controlled so that between about 35% to about 70% of the flow is through the catalytic channels with most preferred catalyst structures having about 50% of the flow through the catalytic channels. In cases where the catalyst structures of the invention are characterized solely by the presence of catalytic channels having a smaller average Dₕ than the non-catalytic channels, the reaction mixture flow distribution is controlled such that the open frontal area of the catalytic channels represents from about 20% to about 80% of the total open frontal area, while the catalytic and non-catalytic channels are configured such that the ratio of the average Dₕ of the catalytic channels to the average Dₕ of the non-catalytic channels is smaller than the ratio of open frontal area of the catalytic channels to the open frontal area of the non-catalytic channels. As used above, open frontal area refers to the cross-sectional area of channels of a given type, i.e., catalytic or non-catalytic averaged over the catalyst structure in question; the cross-sectional area being the area open to reaction mixture flow in a channel measured perpendicular to the reaction mixture flow.

For catalyst structures of the invention characterized solely by the presence of catalytic channels having a higher h than the non-catalytic channels, the ratio h(cat)/h(non-cat) is desirably greater than about 1.5 when the catalytic channels represent from about 20% to about 80% of the total open frontal area in the catalyst structure. Preferred catalytic structures of this type have h(cat)/h(non-cat) ratios in the range of about 1.5 to about 7.

In a preferred aspect, the present invention is directed to catalyst structures which are uniquely useful in the catalytic combustion or partial combustion of a fuel. These catalyst structures are typically monolithic in nature and comprise a heat resistant support material composed of a plurality of common walls which form a multitude of adjacently disposed longitudinal channels for passage of a combustible mixture, e.g., a fuel in gaseous or vaporous form mixed with an oxygen-containing gas such as air. The adjacently disposed channels are designed so that at least a portion of the channels are coated on at least a part of their interior surface with a catalyst suitable for oxidizing the combustible mixture, that is, catalyst-coated channels, and the remaining channels are not coated with catalyst on their interior surface, that is, catalyst-free channels, such that the interior surface of the catalyst-coated channels are in heat exchange relationship with the interior surface of adjacent catalyst-free channels. In this preferred aspect of the invention, the above-described catalyst structures are characterized by the presence of catalyst-coated channels or catalytic channels which differ in configuration from the catalyst-free channels or non-catalytic channels in one or more of the critical respects described above such that the desired combustion or oxidation reaction is promoted in the catalytic channels while it is substantially suppressed in the non-catalytic channels. This extra element of control of the reaction coupled with the enhanced heat transfer which is obtained allows the catalytic combustion process to be operated over a wider range of operating parameters, such as linear velocity, inlet gas temperature and pressure.

In this preferred aspect of the invention, the catalyst structure is suitably a platinum group metal-based catalyst on a ceramic or metal monolith. The monolithic support is assembled such that the catalytic and non-catalytic channels extend in a longitudinal direction from one end of the support to the other, thus enabling the combustible gas to flow from end to end through the length of the channels. The catalytic channels, which have catalyst coated on at least a portion of their interior surfaces, need not be coated along their entire length. Further, the channels not coated with catalyst or non-catalytic channels have no catalyst on their interior walls or an inactive or very low activity coating on their walls.

The support materials suitably employed in the catalyst structures may be any conventional heat resistant, inert material such as a ceramic, heat resistant inorganic oxides, intermetallic materials, carbides, nitrides or metallic materials. The preferred supports are high temperature resistant intermetallic or metallic materials. These materials are strong yet malleable, may be mounted and attached to surrounding structures more readily and offer more flow capacity, per unit of cross-sectional area, due to walls which are thinner than can be readily obtained in ceramic supports. Preferred intermetallic materials include metal aluminides, such as nickel aluminide and titanium aluminide, while suitable metallic support materials include aluminum, high temperature alloys, stainless steels, aluminum-containing steels and aluminum-containing alloys. The high temperature alloy may be a nickel or cobalt alloy or other alloy rated for the required temperature service. If heat resistant inorganic oxides are employed as the support material they are suitably selected from silica, alumina, magnesia, zirconia and mixtures of these materials.

The preferred materials are aluminum-containing steels such as those found in U.S. Patent Nos. 4,414,023 to Aggen et al., 4,331,631 to Chapman et al., and 3, 969,082 to Cairns et al. These steels, as well as others sold by Kawasaki Steel Corporation (River Lite 2-5- SR), Vereinigte Deutchse Metallwerke AG (Alumchrom I RE), and Allegheny Ludlum Steel (Alfa-IV), contain sufficient dissolved aluminum so that, when oxidized, the aluminum forms alumina whishers, crystals, or a layer on the steel's surface to provide a rough and chemically reactive surface for better adherence of the catalyst or of a washcoat for the catalyst.

For catalyst structures in this preferred aspect of the invention, the support material, preferably metallic or intermetallic, may be fabricated using conventional techniques to form a honeycomb structure, spiral rolls or stacked patterns of corrugated sheet, -sometimes inter-layered with sheets which may be flat or of other configuration, or columnar or other configuration which allow for the presence of adjacent longitudinal channels which are designed to present flow channels in accordance with the design criteria set forth above. If intermetallic or metallic foil or corrugated sheet is employed, the catalyst will be applied to only one side of the sheet or foil or in some cases the foil or sheet will remain uncoated depending on the catalyst structure design chosen. Applying the catalyst to only one side of the foil or sheet, which is then fabricated into the catalyst structure, takes advantage of the integral heat exchange concept, allowing heat produced on the catalyst to flow through the structure wall into contact with the flowing gas at the opposite non-catalytic wall thereby facilitating heat removal from the catalyst and maintaining the catalyst temperature below the temperature for complete adiabatic reaction. In this regard, the adiabatic combustion temperature is the temperature of the gas mixture if the reaction mixture reacts completely and no heat is lost from the gas mixture.

In many cases for catalyst structures employed in combustion processes, it may be useful to apply a washcoat to the support wall before depositing the catalyst to improve the stability and performance of the catalyst. Suitably this washcoat may be applied using an approach such as is described in the art, e.g., the application of gamma-alumina, zirconia, silica, or titania materials (preferably sols) or mixed sols of at least two oxides containing aluminum, silicon, titanium, zirconium, and additives such as barium, cerium; lanthanum, chromium, or a variety of other components. For better adhesion of the washcoat, a primer layer can be applied containing hydrous oxides, such as a dilute suspension of pseudo-boehmite alumina, as described in U.S. Patent No. 4,279,782 to Chapman et al. The primed surface may be coated with a gamma-alumina suspension, dried, and calcined to form a high surface area adherent oxide layer on the metal surface. Most desirably, however, is the use of a zirconia sol or suspension as the washcoat. Other refractory oxides, such as silica and titania, are also suitable. Most preferred for some platinum group metals, notably palladium, is a mixed zirconia/silica sol where the two have been mixed prior to application to the support.

The washcoat may be applied in the same fashion one would apply paint to a surface, e.g., by spraying, direct application, dipping the support into the washcoat material, etc.

Aluminum structures are also suitable for use in this invention and may be treated or coated in essentially the same manner. Aluminum alloys are somewhat more ductile and likely to deform or even to melt in the temperature operating envelope of the process. Consequently, they are less desirable supports but may be used if the temperature criteria can be met.

For ferrous metals containing aluminum, the sheet may be heat treated in air to grow whiskers at the surface that increase adhesion of subsequent layers or provide increased surface area for direct application of a catalyst. A silica, alumina, zirconia, titania, or refractory metal oxide washcoat may then be applied by spraying onto the metal foil a solution suspension, or other mixture of one or more materials selected from alumina, silica, zirconia, titania and a refractory metal oxide, and drying and calcining to form a high surface area washcoat. The catalyst can then be applied, again such as by spraying, dripping or coating a solution, suspension, or mixture of the catalytic components onto the washcoats on the metal strip.

The catalytic material may also or alternatively be included in the washcoat material and coated onto the support thereby partially eliminating the separate catalyst inclusion step.

In the catalytic combustion application, where a substantial portion of the combustion is carried out after the gas exits the catalyst, the catalyst structure may be sized to achieve a gas temperature exiting the catalyst no more than 1000°C, preferably in the range of 700°C and 950°C. The preferred temperature is dependent on the fuel, the pressure and on the specific combustor design. The catalyst can incorporate a non-catalytic diffusion barrier layer on the catalytic material such as that described in U.S. Patent No. 5,232,357.

The catalytic metal content of the composite, i.e., the catalyst structure, is typically quite small, e.g., from 0.01% to about 15% by weight, and preferably from 0.01% to about 10% by weight. Although many oxidation catalysts are suitable in this application, Group VIII noble metals or platinum group metals (palladium, ruthenium, rhodium, platinum, osmium, and iridium) are preferred. More preferred are palladium (because of its ability to self-limit combustion temperatures) and platinum. The metals may be used singly or in mixtures. Mixtures of palladium and platinum, are desirable since they produce a catalyst having the temperature limiting capabilities of palladium, although at a different limiting temperature, and the mixture is less susceptible to deactivation by reaction with impurities in the fuel or by reaction with the catalyst support

The platinum group metals or elements may be incorporated onto the support employed in the catalyst structure of the invention by a variety of different methods using noble metal complexes, compounds, or dispersions of the metal. The compounds or complexes may be water of hydrocarbon soluble. The metal may be precipitated from solution. The liquid carrier generally needs only to be removable from the catalyst carrier by volatilization or decomposition while leaving the metal in a dispersed form on the support.

Suitable platinum group metal compounds are, for example, chloroplatinic acid, potassium platinum chloride, ammonium platinum thiocyanate, platinum tetrammine hydroxide, platinum group metal chlorides, oxides, sulfides, and nitrates, platinum tetrammine chloride, platinum ammonium nitrite, palladium tetrammine chloride, palladium ammonium nitrite, rhodium chloride, and hexamine iridium chloride. If a mixture of metals is desired, they may be in water soluble form, for example, as amine hydroxides or they may be present in such forms as chloroplatinic acid and palladium nitrate when used in preparing the catalyst of the present invention. The platinum group metal may be present in the catalyst composition in elemental or combined forms, e.g., as an oxide or sulfide. During subsequent treatment such by calcining or upon use, essentially all of the platinum group metal is converted to the elemental form.

Additionally, by placing a more active catalyst, preferably palladium, on the portion of the catalyst structure which first contacts the combustible gas, the catalyst will "light off' more easily and yet not cause "hot spots" in the latter regions of the structure. The leading portion may be more active because of higher catalyst loadings, higher surface area, or the like.

'In the catalytic combustion application, the catalyst structure of the invention should be made in such a size and configuration that the average linear velocity of the gas through the longitudinal channels in the catalyst structure is greater than about .02 m/second throughout the catalytic structure and no more than about 80 m/second. The lower limit is larger than the flame front speed for methane in air at 350°C and the upper limit is a practical one for the type of supports currently commercially available. These average velocities may be somewhat different for fuels other than methane. Slower burning fuels may permit use of a lower minimum and maximum space velocity.

The average size of the channels employed in the catalyst structure can vary widely dependent on the nature of the reaction mixture. For catalytic combustion, suitable catalyst structures contain about 50 to about 600 channels per square inch. Preferably, the catalyst structure will contain from about 150 to about 450 channels per square inch.

The catalytic combustion process of the invention employing the catalyst structure of the invention may be used with a variety of fuels and at a broad range of process conditions.

Although normally gaseous hydrocarbons, e.g., methane, ethane, and propane, are highly desirable as a source of fuel for the process, most fuels capable of being vaporized at the process temperatures discussed below are suitable. For instance, the fuels may be liquid or gaseous at-room temperature and pressure. Examples include the low molecular weight hydrocarbons mentioned above, as well as butane, pentane, hexene, heptene, octane, gasoline, aromatic hydrocarbons, such as benzene, toluene, ethylbenzene, xylene, naphthas, diesel fuel, kerosene, jet fuels, other middle distillates, heavy distillate fuels (preferably hydrotreated to remove nitrogenous and sulfurous compounds), oxygen-containing fuels, such as alcohols including methanol, ethanol, isopropanol, butanol, or the like; ethers, such as diethylether, ethyl phenyl ether, MTBE, etc. Low-BTU gases, such as town gas or syngas, may also be used as fuels.

The fuel is typically mixed into the combustion air in an amount to produce a mixture having a theoretical adiabatic combustion temperature or Tad greater than the catalyst or gas phase temperatures present in the catalysts employed in the process of the invention. Preferably the adiabatic combustion temperature is above 900°C, and most preferably above 1000°C. Non-gaseous fuels should be vaporized prior to their contacting the initial catalyst zone. The combustion air may be compressed to a pressure of 500 psig. or more. Stationary gas turbines often operate at pressures in the vicinity of 150 psig.

The process of the invention can be carried out in a single catalytic reaction zone employing the catalyst structure of the invention or in multiple catalytic reaction zones, usually 2 or 3, using catalyst structures designed specifically for each catalytic stage. In most cases the catalytic reaction zone will be followed by a homogeneous combustion zone in which the gas exiting from the earlier catalytic combustion zone is combusted under non-catalytic, non-flame conditions to afford the higher gas temperature, e.g., temperatures in the range of 1000-1500°C, required by gas turbines.

The homogeneous combustion zone is sized to achieve substantially complete combustion and to reduce the carbon monoxide level to the desired concentration. The gas residence time in the post-catalyst reaction zone is 2 to 100 ms, preferably 10 to 50 ms.

An additional aspect of the invention, which is particularly suited to the catalytic combustion or partial combustion of a fuel, relates to improved catalytic reaction systems and/or processes for catalytic combustion wherein a flameholder or other means for inducing gas recirculation into the homogeneous combustion zone downstream of a catalytic structure employing integral heat exchange, preferably the improved catalyst structures of the present invention, is used to further broaden the range of operating conditions at which the combustion can take place with little or no concomitant formation of NOₓ. The flameholder concept is well known in the conventional non-catalytic combustion art, e.g., see Lovett et al., "Emissions and Stability Characteristics of Flameholders for Lean-Premixed Combustion," *ASME* Publication No. 92-GT-120, presented at the International Gas Turbine and Aeroengine Congress and Exposition, Cologne, Germany, June 1-4, 1992. Further, German Patentschrift DE 42 02 018 Cl, published April 29, 1993, teaches the use of a flameholder downstream of a conventional partial combustion catalyst to expand the stability area of the catalytic combustion. However, there has been no teaching of the use of a flameholder or similar gas recirculation inducing means in the homogeneous combustion zone downstream from a catalyst employing integral heat exchange nor further the important benefits which can flow from such use.

In fact, in past practice, flameholders have generally been applied to rich F/A mixtures at low temperatures, in many cases with the use of an additional ignition device to initiate combustion. In the case of the present invention, equipping the homogeneous combustion zone downstream of a catalyst structure employing integral heat exchange with a flameholder or similar gas recirculation inducing means allows the flameholder to act in a passive fashion to stabilize the homogeneous combustion in the region of recirculation downstream from the flameholder, with the result being that stabilized homogeneous combustion can be obtained at lower catalyst structure outlet temperatures and/or leaner F/A ratios. The ability to operate at lower catalyst structure outlet temperatures has practical benefits to the system in that enhanced catalyst lifetimes can be obtained and/or the size of the catalytic structure can be reduced while still obtaining essentially complete combustion (minimal unburned hydrocarbons and CO being present in the combustion gases) with little or no NOₓ formation.

When the flameholder or other means for inducing gas recirculation into the homogeneous combustion zone is combined with the use of a catalyst structure employing integral heat exchange such as that described in U.S. Patent No. 5,250,489 (the disclosure of which is herewith incorporated by reference) or the improved catalyst structures of the present invention, which also utilize integral heat exchange, the degrees of freedom in operating parameters for combustion or partial combustion processes are even further enhanced since integral heat exchange inherently provides lower catalyst structure outlet temperatures and the addition of the flameholder promotes homogeneous combustion at these lower catalyst structure outlet temperatures. In its most general terms, this aspect of the invention employs any means for inducing gas recirculation in the homogeneous combustion zone including conventional flameholders and the use of homogeneous combustion zones where the cross-sectional area defined by the containment wall or walls of the homogeneous combustion zone is changed or varied over the length of the combustion zone in the direction of partially-combusted gas flow such that turbulence and recirculation are induced into the gas flow by the restrictions and/or expansions in areas the gas flow encounters as it moves through the zone. In the latter case, there is typically a step change in the cross-sectional area of the homogeneous combustion zone which causes a level of recirculation in the flowing gas such that the residence time of the gas in the zone is increased sufficient to induce and stabilize homogeneous combustion within the homogeneous combustion zone.

The flameholder device is a physical object or a flow pattern that results in gas recirculation that causes an increase in the residence time for some portion of the fuel/air mixture. If the longer residence time is in the range of the ignition delay time for that specific gas mixture and gas temperature, then the gas mixture will ignite and combustion will be stabilized in the recirculation region. The combustion heat and radicals will spread into the main flow path and the combustion wave will spread until the entire flowing fuel/air mixture is combusted. Conventional flameholder devices which are suitable for use in the present invention include a bluff body, a V-gutter, a cone, a perforated plate and a swirler, each of which may be inserted into the homogeneous combustion zone immediately downstream from the outlet end of the catalyst structure. In some cases it is desirable to employ several different flameholder devices in the same combustion zone with the combination of a flameholder device and the use of a homogeneous combustion zone where the cross-sectional area is changed in direction of gas flow being particularly desirable. In any event, to obtain effective gas flow recirculation, the flameholder or combination of flameholders employed suitably provide a geometric flow blockage in the homogeneous combustion zone of from about 5 to about 90 percent, with geometric flow blockages in the range of about 20 to about 70 percent being preferred.

The positioning of the flameholder in the homogeneous combustion zone will depend on. a variety of factors including the temperature of the partially-combusted gas at the catalyst structure outlet, -the F/A ratio of the fuel mixture, the gas flow rate, the type of fuel being combusted, the percent combustion occurring in the catalyst structure and the intensity of mixing or extent of gas recirculation obtained using the flameholder. Typically, the flameholder will be positioned at a point in the homogeneous combustion zone downstream of the catalyst structure outlet such that the average residence time of the partially-combusted fuel in the region of recirculation created by the flameholder approximates the ignition delay time for the specific gas mixture and gas temperature present in the homogeneous combustion zone. Typically, the flameholder will be positioned from about 0.1 to about 50 cm downstream from the outlet end of the catalyst structure and preferably from about 0.5 to about 20 cm downstream from the catalyst structure outlet. With the flameholder positioned as described above, the theoretical adiabatic combustion temperature or Tad of the fuel/air mixture fed to the catalyst structure is typically between about 900 to 1000°C and, preferably, in the low end of that range, for example, 900 to 1300°C. Further, the advantage achieved by the flameholder in stabilizing combustion in the homogeneous combustion zone is most apparent when between about 20 and 70 percent of the fuel in the combustible mixture is combusted in the catalyst structure to afford an outlet temperature for the partially-combusted, gaseous mixture flowing out of the outlet end of the catalyst structure of between about 700 and about 1000°C.

Referring now to the drawings, FIGS. 1 and 2 depict end views of repeating units of two conventional catalyst structures employing integral heat exchange. The repeating units shown would appear in a stacked or layered pattern in the complete catalyst structure. In FIG. 1 the support is made up of two metallic sheets or strips one (10) having an undulating or wavy corrugation pattern and the other (12) being flat. The crests and valleys formed by the corrugation extend in a longitudinal direction over the width of the sheet and nest against the flat sheets both above and below the corrugated sheet to form straight longitudinal channels (14 and 16) which extend over the width of the stacked or nesting sheets. The undulating or sinusoidal corrugation pattern shown here is only representative. The corrugation can be sinusoidal, triangular, or any other conventional structure. The bottom side of the undulating sheet (10) and the top side of the flat sheet (12) are coated with catalyst or washcoat plus catalyst (18) such that when the sheets are stacked together as shown, channels coated with catalyst (14) are in integral heat exchange with channels not coated with catalyst (16). As noted above, the catalytic channels (14) and non-catalytic channels (16) formed are essentially straight and of unaltered cross-sectional area. This structure provides catalytic and non-catalytic channels wherein the ratio of the average Dₕ of the catalytic channels to average Dₕ of the non-catalytic channels is 1 and the h(cat)/h(non-cat) ratio is also 1.

The repeating unit shown in FIG. 2 is comprised of two corrugated metallic sheets (20 and 22) having a herringbone corrugation pattern extending in a longitudinal direction over the length of the sheets. One of the corrugated sheets (22) is coated with catalyst (24) on its top side while the other corrugated sheet is coated with catalyst on its bottom side such that when the sheets are stacked together in non-nesting fashion a catalyst-coated channel (26) is formed in integral heat exchange with a catalyst-free channel (28).

FIG. 3 shows further detail of the metallic sheets having herringbone corrugation pattern which are suitably employed in the structure shown in FIG. 2 above or in structures of the invention when herringbone corrugations are used to induce tortuosity into the catalytic channels. As can be seen from the side and top or planar views represented in FIG. 3 the sheet is corrugated to form peaks (30) and valleys (32) which in turn form the herringbone pattern along the width of the sheet. The triangular corrugation pattern shown in FIGS. 2 and 3 is only for representation. The corrugation can be triangular, sinusoidal or any other corrugated structure envisioned in the art.

The non-nesting nature of the corrugated sheets and the effect the herringbone corrugation pattern, shown in FIG. 2, has on the shape of the catalytic and non-catalytic channels at various points along their length is further illustrated in FIGS. 3A, 3B and 3C. These Figures show cross-sectional views of the repeating unit taken from the end view (FIG. 3A - which is the same as FIG. 2) and at incremental points on the longitudinal axis of the channels (FIGS. 3B and 3C) where the different directional orientations of the stacked herringbone corrugations cause the peaks and valleys formed by the corrugations in each sheet to change position relative to the position of the peaks and valleys of the corrugated sheet directly above and below it in the repeating unit. In FIG. 3A, the channels, both catalytic (26) and non-catalytic (28) have a repeating V-shaped cross-section wherein FIG. 3B the change in channel wall orientation caused by different directional orientations in the peaks and valleys of adjacent herringbone patterned corrugations results in channels (26 and 28) which are rectangular in cross-sectional area. Finally, in FIG. 3C, at the point where the peaks and valleys defining the herringbone corrugation pattern of a given sheet come into contact with the respective valleys and peaks of the herringbone patterned corrugations of sheets directly above and below the sheet in question, that is, the point where the herringbone corrugations on adjacent sheets cross-over one another, the catalytic channels (26) and non-catalytic channels (28) have a diamond shaped cross-sectional area. Of course, this pattern of changing cross-sectional shape of the channels will repeat itself over and over along the entire length of the channel defined by the non-nesting herringbone corrugations. In this case, even thought the non-nesting herringbone patterned corrugations result in channels which have a variable cross-sectional area along their length, the catalytic and non-catalytic channels show identical variation along their length. As a result, the structure shown in FIG. 2 provides catalytic and non-catalytic channels wherein the average Dₕ of the catalytic channels is equal to the average Dₕ of the non-catalytic channels and where the h(cat)/h(non-cat) ratio is equal to 1.

FIG. 4 represents an end view of a repeating unit of a catalyst structure of the invention wherein a series of metallic sheets of various configurations are employed in a stacked pattern to afford catalytic channels which differ in configuration from the non-catalytic channels in accordance with the invention. This repeating unit is made up of a combination of two flat sheets (40), one corrugated sheet (42) a straight corrugation pattern forming straight channels, and two corrugated sheets (44) having herringbone corrugation pattern. Catalytic channels (46) and non-catalytic channels (48) are formed by selectively coating one side of the two flat sheets and one side of one of the corrugated sheets with catalyst (50). As can be seen from the Figure, non-catalytic channels are formed from the stacking of the flat sheets with the straight channel sheet to provide large opened channels. In contrast, the catalytic channels are formed from herringbone corrugation foils or sheets stacked in non-nesting fashion between two flat sheets such that channels having tortuous flow paths and smaller Dₕ are provided by the structure. This structure having the dimensions given in Example 2, below, provides catalytic and non-catalytic channels wherein the ratio of average Dₕ of the catalytic channels to the average Dₕ of the non-catalytic channels is 0.66 and the h(cat)/h(non-cat) ratio is 2.53. In that case, the ratio of heat transfer area between catalyst-coated and catalyst-free channels divided by the total channel volume in the structure is 0.30 mm⁻¹.

FIG. 5 depicts a preferred catalyst structure according to the invention by means of an end view of the repeating unit which is stacked to form the catalyst structure. This repeating unit is made up of three different types of corrugated metallic sheet (52, 54a and 54b). The first type of corrugated sheet (52) is essentially a flat sheet in which the extended flat regions are separated periodically by sharp peaked corrugations with the peaked corrugations extending straight across the foil forming a straight corrugation pattern. The second type of corrugated sheet (54a and 54b) is made up of a series of corrugations in the herringbone pattern. In the repeating unit shown, two of the herringbone corrugated sheets are stacked in non-nesting fashion on top of the sheet having wide regions of flat sheet separated by sharp peaked corrugations. In addition, a second flat sheet with sharp peaked corrugations is stacked on top of the top corrugated sheet in the non-nesting corrugated herringbone pattern stack. Catalyst (56) is coated on the bottom of each of the flat sheets with sharp peaked corrugations and on the top of the bottom corrugated herringbone pattern sheet thereby forming catalytic channels (58a and 58b) having small hydraulic diameters and tortuous flow channels and non-catalytic channel (60) which is a larger more open channel of substantially straight configuration. With this preferred catalyst structure constructed to have the dimensions given in Example 3, below, the ratio of the average Dₕ of the catalytic channels to the average Dₕ of the non-catalytic channels is 0.41 while the h(cat)/h(non-cat) ratio is 1.36. Further, the ratio of heat transfer area between catalytic and non-catalytic channels, divided by the total channel volume in this preferred structure having the dimensions given in Example 3, is 0.74.

The preferred structure depicted in FIG. 5 can be readily modified to increase the number and tortuosity of the catalytic channels by inserting additional corrugated sheets having a herringbone corrugation pattern between the two flat sheets with sharp peaked corrugations. If additional corrugated sheets are inserted in the repeat unit (stacked in non-nesting fashion with the two sheets shown in the Figure) they can be coated on one side of the other or remain uncoated depending on the catalyst structure desired.

FIG. 6 illustrates the repeat unit of another catalyst structure of the invention viewed from its inlet end. As depicted, the support is made up of two essentially flat metallic sheets (62) wherein the horizontal flat regions are periodically divided by vertical strips to form large open regions and three corrugated metallic sheets having a herringbone corrugation pattern (64, 66 and 68) which are stacked in non-nesting fashion between the two essentially flat sheets. These three corrugated sheets differ in the severity of the corrugations, that is, the number of corrugations per unit of width, with the top and middle corrugated sheets (64 and 66) having a more severe corrugation pattern than the bottom corrugated sheet (68). The catalyst (70) is coated on the bottom of the two essentially flat sheets (62) and on the bottom of the top corrugated sheet (64) and top of the bottom corrugated sheet (68) with the result being as large open non-catalytic channel (72) which is essentially straight in configuration and three catalytic channels (74, 76 and 78) which have very small average Dₕ's and configurations which create tortuous flow paths. For this structure in which sheet (62) has a height of 1.6 mm and a flat region of 3.3 mm; sheet (68) has a height of 0.41 mm and a peak-to-peak period of 0.66 mm; sheet (66) has a height of 1.1 mm and a peak-to-peak period of 0.33 mm; and sheet (64) has a height of 0.69 mm and a peak-to-peak period of 0.31 mm, the ratio of average Dₕ of the catalytic channels to average Dₕ of the non-catalytic channels is 0.15 and the h(cat)/h(non-cat) ratio is 2.72. In this case the ratio of heat transfer area between the catalyst-coated and catalyst-free channels divided by the total channel volume in the structure is 0.91 mm⁻¹.

Based on the design criteria set forth above, one skilled in the art will be able to construct a variety of catalyst structures which are within the scope of the invention. Other possible structures are shown in FIGS. 7 and 8 where end views of repeat units for the structures are depicted. In FIG. 7, corrugated metal sheets (80 and 82) having a herringbone corrugation pattern are stacked in non-nesting fashion between a corrugated metal sheet (84) having crests and valleys extending in a longitudinal straight direction over the length of the sheet. Catalyst (86) is coated on the bottom of the top corrugated sheet (80) and the top of the bottom corrugated sheet (82) such that catalytic channels (88) of small average Dₕ and significant tortuosity are formed in integral heat exchange with larger more open catalyst-free channels (90) which present essentially straight flow channels.

In FIG. 8, three corrugated metallic sheets (92, 94 and 96), having a herringbone corrugation pattern are stacked in non-nesting fashion between a straight channel corrugated metal sheet (98) of similar configuration to the corrugated sheet used in the structures of FIG. 7. Catalyst (100) is coated on the bottom of the top corrugated sheet (92) and the top of the bottom corrugated sheet (96) to form catalyst-coated channels (102) having a small average Dₕ and tortuous flow paths in heat exchange relationship with larger, open catalyst-free channels (104) which have essentially straight flow paths.

FIGS. 9 and 10 depict schematic representations of the reaction system according to the invention wherein the homogeneous combustion zone downstream of the catalyst structure is equipped with a flameholder to stabilize combustion of a partially-combusted fuel/air mixture within the homogeneous combustion zone. In FIG. 9, the reaction system is made up of a combustor (110) containing a catalytic section or zone (112) and a homogeneous combustion zone (114) with the fuel/air mixture (116) being fed to the inlet end of the catalytic section where partial combustion of the fuel occurs in the presence of the catalyst to afford a heated, partially-combusted, gaseous mixture which flows from the outlet end of the catalytic-section through the homogeneous combustion zone where the residual fuel is completely combusted under non-catalytic conditions. In this case a hemispherical disk flameholder (118) is positioned in the homogeneous combustion zone immediately downstream of the catalytic section outlet such that some portion of the heated, partially-combusted, gaseous mixture flowing past the hemispherical disk flameholder is recirculated in the region of the homogeneous combustion zone just downstream of the flameholder and non-catalytic combustion is stabilized in the region of recirculation.

FIG. 10 similarly shows combustor (120) comprised of a catalytic section (122) and a homogeneous combustion zone (124) downstream of the catalytic section with the fuel/air mixture (126) being introduced into the inlet end of the-catalytic section. In this case the flameholder (128) positioned immediately downstream of the catalytic section is a V-gutter flameholder which effects recirculation of the heated, partially-combusted, gaseous mixture leaving the catalytic section in a manner similar to that obtained with the hemispherical disk flameholder described above.

In both cases described above, the catalytic section can be any catalytic structure employing integral heat exchange including the structures described in U.S. Patent No. 5,250,489 but preferably is one of the improved catalyst structures of the present invention which are described in detail above. With either reaction system employing a flameholder as described above, temperature sensors can be positioned at various points downstream of the flameholder to monitor the temperature profile of the hot gases in the homogeneous combustion zone.

Various conventional flameholders are depicted in end view and cross-sectional view in FIGS. 11A through 14B. FIGS. 11A and 11B show a cone-type flameholder (130) affixed to the sidewall of the homogeneous combustion zone (132) via support struts or bars (134). FIGS. 12A and 12B depict a V-gutter-type flameholder (140) attached to the sidewall of the homogeneous combustion zone (142) by support bars (144). FIGS 13A and 13 B show a perforated, plate-type flameholder (150) which abuts against and is attached to the sidewall of the homogeneous combustion zone (152). This perforated plate is equipped with a multiplicity of openings or flow passages (154) for passage of the heated, partially-combusted gas flow through the homogeneous combustion zone. Finally, FIGS 14A and 14B show a swirler-type flameholder having a series of swirl vanes (160), which are secured inside the sidewall of the homogeneous combustion zone (162) via support plates or bars (164) and bluff body (166) which may be solid or a hollow shell.

### EXAMPLES

The following examples demonstrate some of the advantages achieved by the use of the inventive catalyst structure as compared to conventional catalyst structures employing integral heat exchange.

### Example 1

Using the conventional catalyst structure shown in FIG. 2, a catalyst was prepared and tested in the combustion of a gasolinetype fuel as follows:

A SiO₂/ZrO₂ powder was prepared by first mixing 20.8 g of tetraethylorthosilicate with 4.57 cc of 2 mM nitric acid and 12.7 g of ethanol. The mixture was added to 100 g of zirconia powder having a specific surface are of 100 m²/gm. The resulting solid was aged in a sealed glass container for about a day and dried. One portion was calcined in air at 500°C and another portion was calcined in air at 1000°C.

A sol was prepared by mixing 152 g of the SiO₂/ZrO₂ powder calcined at 1000°C and 15.2 g of the SiO₂/ZrO₂ powder calcined at 500°C with 3.93 g of 98% H₂SO₄ and 310 cc of distilled water. This mixture was milled using ZrO₂ grinding media for eight hours to product a SiO₂/ZrO₂ sol.

A Fe/Cr/Al alloy (Fe/20%Cr/5%Al) foil strip 76 mm wide was corrugated in a herringbone pattern to a corrugation height of 1.20 mm and a peak to peak period of 2 mm and the herringbone pattern had channel lengths of 20 mm and a channel angle of 6° and forms a monolithic structure with about 185 cells per square inch. This foil was heat treated in air at 900°C to form a rough oxide coated surface.

The SiO₂/ZrO₂ sol was sprayed onto one side of the herringbone corrugated foil to a thickness of about 40 micrometers and the coated foil calcined in air at 950°C. Pd(NH₃)₂(NO₂)₂ and Pt(NH₃)₂(NO₂)₂ was dissolved in water and an excess of nitric acid to form a solution containing about 0.1 g Pd/ml and a Pd/Pt ratio of 6; this solution was sprayed onto the SiO₂/ZrO₂ coated corrugated to form a final Pd loading of about 0.25 g Pd/g of SiO₂/ZrO₂ and calcined in air at 950°C.

A strip of the above foil was folded against itself to place the catalyzed side of the foil facing itself and the structure rolled to form a spiral monolithic structure of 50 mm diameter. This catalyst (rolled into a spiral wound structure with 50 mm diameter) was installed in the test rig described above. Thermocouples were installed to measure the substrate temperature and to measure temperatures of the gas downstream of the catalyst. In addition, a water-cooled gas sampling probe was installed in the reactor to measure the composition of the gas stream at the position 25 cm downstream of the catalyst. The test sequence was as follows:
1. Set air flow to that consistent with gas turbine idle condition.
2. Set air temperature at value in range of air temperature for gas turbine cycle at idle.
3. Increase fuel to flow necessary for adiabatic combustion temperature of 1200°C.
4. Increase air temperature to find upper limit of catalyst operation as determined by overheating of the catalyst. In this test procedure, the upper limit of catalyst operating temperature was taken at 1050°C substrate temperature.
5. Similarly decrease the air temperature until the lower limit of catalyst operation is found as determined by an increase of emissions above the target value. In this test procedure, the lower limit was taken as the inlet air temperature when the CO emissions at 25 cm post-catalyst exceeded 5 ppm by volume (dry).
6. The procedures of steps 1 through 5 were repeated with the air flow typical of the gas turbine operated at full load conditions.

Specification indolene clear gasoline was used as the fuel. This is a standard unleaded regular gasoline used for emissions qualification. The fuel was injected into the main flow stream of heated air through a spray nozzle and vaporized prior to passing through the static mixer to form a uniform fuel/air mixture at the catalyst inlet. Fuel and air flow was continuously measured in real time and controlled through automatic feedback control.

The results of the test of the catalyst structure including test conditions employed are shown in Table 1 below.

**Table 1**

| Condition | Air Flow | Pressure | Tad(*C) | Inlet Temperature at Op Window | |
|---|---|---|---|---|---|
| | (SLPM) | (atm) | | Bottom (°C) | Top (°C) |
| Idle | 291 | 1.3 | 1150 | 230 | 400 |
| | | | 1200 | 220 | 260 |
| | | | 1250 | 220 | 220 |
| Full Load | 2127 | 2.9 | 1200 | 540 | >620 |
| | | | 1300 | 420 | 570 |

Summary: At idle conditions, this catalyst will operate at a F/A ratio equivalent to an adiabatic combustion temperature of 1150°C over an inlet temperature range of 230 to 400°C. At 1200°C Tad, this inlet temperature range has narrowed to 220-260°C and at 1250°C the catalyst will not operate without overheating.

At full load, this catalyst system operates reasonably well with an operating range of 540 to >620°C at 1200°C Tad, and 420 to 570°C at 1300°C.

This catalyst system does not have a wide operating range at idle and cannot be used in a turbine that must operate from idle to full load, unless the fuel/air ratio is controlled to a very narrow range.

### Example 2

To minimize combustion of fuel in the non-catalytic channels at low air flow rates, the catalyst structure shown in FIG. 4 was evaluated using the same fuel as employed in Example 1. The straight channel corrugation had a corrugation height of 1.65 mm and was approximately triangular with a peak-to-peak period of 3.90 mm. The herringbone corrugation foils were similar to that described in Example 1, except the foils had height of 0.76 mm and 0.91 mm and peak-to-peak period of 1.84 and 2.45 for the two foils. The catalytic coating (Pd-Pt/SiO₂/ZrO₂) was prepared and applied as described in Example 1. The performance of this catalyst structure using the same procedure described in Example 1 is shown in Table 2.

**Table 2**

| Condition | Air Flow | Pressure | Tad(°C) | Inlet Temperature at Op Window | |
|---|---|---|---|---|---|
| | (SLPM) | (atm) | | Bottom (°C) | Top (°C) |
| Idle | 291 | 1.3 | 1200 | 460 | >500 |
| | | | 1300 | 290 | 550 |
| Full Load | 2127 | 2.9 | 1200 | 610 | >620 |
| | | | 1300 | 510 | 610 |

Summary: This unit has substantially better performance at idle than the catalyst of Example 1. At these very low air flow rates, the catalyst substrate does not overheat so readily. However, the operating window at full load has decreased and the unit does not provide the inlet temperature operating range at 1200 and 1300°C Tad required for optimum performance. Clearly, the use of open and large non-catalytic channels allows the catalyst to operate better at very low mass velocities but this particular design appears to have limited heat exchange between the catalytic channels and the non-catalytic channels. This results in a low outlet gas temperature from the catalyst at high mass flows and less than optimum performance at full load conditions.

### Example 3

The catalyst structure of FIG. 5 was prepared and tested according to the procedures described in Example 1. In the catalyst structure tested, the herringbone corrugation foils were similar to that described in Example 1, except the foils had heights of 0.76 mm and 1.2 mm and pitches of 1.84 and 2.90 and a chevron angle of 6° for the two herringbone foils and the straight corrugation peaked foil had a height of 1.63 mm, a peak-to-peak period of 4.52 mm and a flat region length of 3.7 mm. Again, the catalyst was Pd-Pt/SiO₂/ZrO₂ prepared in accordance with Example 1, and it was applied as shown in FIG. 5. The operating window conditions and test results are shown below using the Indolene Clear gasoline in Table 3.

**Table 3**

| Condition | Air Flow | Pressure | Tad(°C) | Inlet Temperature at Op Window | |
|---|---|---|---|---|---|
| | (SLPM) | (atm) | | Bottom (°C) | Top (°C) |
| Idle | 291 | 1.3 | 1200 | 390 | >500 |
| | | | 1300 | 280 | 490 |
| Full Load | 2127 | 2.9 | 1200 | 570 | >620 |
| | | | 1300 | 470 | 620 |

Summary: The catalyst structure has very wide operating windows at both idle and full load condition. At idle, this catalyst can operate over an inlet temperature range of 160°C at 1200°C Tad and over a range of 210°C at 1300°C Tad. At full load the range is >50°C at 1200°C. These operating windows are sufficient Tad and is >50°C at 1200°C Tad and >150°C at 1300°C. These operating windows are sufficient to make this catalyst system viable for use in a practical gas turbine. Comparison to the conventional technology of Example 1 shows that the catalyst of Example 3 can operate from 1200 to 1300°C Tad range at both idle and full load while the conventional catalyst of Example 1 could only operate from 1150°C to 1200°C Tad and only over very narrow catalyst inlet temperatures at idle. In addition, the conventional technology of Example 1 would require very narrow control of fuel/air ratio which may be very difficult and costly. The technology of Example 3 has much broader operating windows and would permit more easy practical application. The operating. range at full load was nearly as wide for the catalyst of Example 3 compared to Example 1.

The following Examples illustrate operation of the reaction system according to the invention where a flameholder is incorporated into the homogeneous combustion zone, as well as some of the advantages attributable to such flameholder.

This invention has been shown both by direct description and by example. The examples are not intended to limit the invention as later claimed in anyway; they are only examples. Additionally, one having ordinary skill in this art would be able to recognize equivalent ways to practice the invention described in these claims. Those equivalents are considered to be within the spirit of the claims invention.

### Examples 4 and 5

A reaction system as illustrated in FIGS. 9 and 10 was set up using a hemispherical disk flameholder (FIG. 9) or a V-gutter flameholder (FIG. 10) and using the general procedure set forth in Example 1 (including catalyst preparation) the flameholder equipped reaction systems were compared to the same reaction system minus a flameholder in the catalytic combustion of indolene gasoline. In each case, the catalyst structure employed was the improved catalyst structure of the invention as depicted in FIG. 5 hereto and temperature sensors were placed downstream of the flameholders or in a similar location in the case where no flameholder was used. For convenience herein the reaction system minus the flameholder will be referred to as Configuration 1, while the system equipped with the hemispherical disk flameholder and the V-gutter flameholder will be designated as Configurations 2 and 3, respectively.

In each test, the air flow was established and the inlet temperature raised to either 400°C or 500°C. Then indolene clear fuel was added to the air via an air assist atomizing nozzle as described in Example 1 above. The fuel-to-air ratio was slowly increased with the actual fuel-to-air ratio being expressed by the adiabatic combustion temperature of the fuel-to-air mixture, that is the temperature that the mixture would attain if all of the fuel were combusted without any os of eat. The fuel-to-air ratio was raised in steps of 50°C from 1050°C.

The data in FIGS. 15 and 6 show the temperature of the gas at a position just downstream of the catalyst or flameholder, as measured by the temperature sensor. As the fuel concentration is increased (the adiabatic combustion temperature or combustor outlet temperature is increased) the temperature profile for these tests show the following:

FIG. 15. For the catalyst only, Configuration 1, the gas temperature is relatively low and increased linearly as the fuel/air mixture (adiabatic combustion temperature) is increased. There is no homogeneous combustion of the fuel/air mixture up to the 7 cm post-catalyst position for this catalyst design and gas velocity. Homogeneous combustion is occurring at some position downstream of the 7 cm temperature sensor.

For Configuration 2, with the hemispherical flameholder after the catalyst, the temperature profile just downstream of the catalyst shows homogeneous combustion, as indicated by the rapid rise in gas temperature at the 7 cm position at a Tad of 1200°C.

FIG. 16 compares the catalyst only, Configuration 1, with the catalyst plus V-gutter flameholder, Configuration 3. Again, the flameholder makes the combustion wave appear at much lower Tad values, in the case of the V-gutter flameholder, it appears at 100°C to 1150°C Tad at a 500°C inlet temperature.

### Example 6

Using the Configurations 1 and 3 and general procedures set forth in Examples 4 and 5 above, a series of combustion runs were carried out to establish the effect, if any, of the addition of a flameholder on the operating window of the catalytic structure depicted in FIG. 5 herein. For purposes of this Example, the operating window is established by the following boundaries:
- Upper limit: Catalyst temperature increases to its maximum.
- Lower limit: Homogeneous combustion does not occur and the fuel is not fully burned before the exit of the combustor. This uncombusted fuel will exit the combustor and produce unacceptably high emissions.
The operating window is measured by holding the adiabatic combustion temperature (or combustor exit temperature) constant and raising the catalyst inlet temperature to determine the oeprating limits as described above. The precise additions or variances to the test procedure described above were as follows:
1. A low catalyst inlet temperature is chosen and the fuel-to-air ratio is set to a selected Tad value such at 1300°C.
2. The catalyst inlet temperature is then slowly increased and the fuel-to-air ratio decreased to keep the Tad constant. At some value of inlet temperature, the emissions at the combustor exit reach the desired value of <10 ppm CO and uncombusted hydrocarbons. This inlet temperature is the operating window bottom.
3. The catalyst inlet temperature is further increased until the catalyst operating temperature reaches its upper limit. The inlet temperature at which the catalyst reaches its upper limit is the operating window top.
The results obtained in the testing are shown in Table 4.

**Table 4**

| CONFIGURATION | INLET TEMPERATURE RANGE AT | |
|---|---|---|
| | 1200°C Tad | 1300°C Tad |
| Configuration 1 | 575 to >650 | 475 to 610 |
| | | |
| Configuration 3 | 510 to >650 | 410 to 610 |

Clearly, the flameholder moves the window bottom to substantially lower temperatures. This would permit the engine to be operated over a much broader range of catalyst inlet temperatures. Also, at a constant inlet temperature, the range of Tad values over which the engine can be operated with low emissions is broader. This will allow the engine to be operated with less precise fuel control. This will lower the cost of the engine and make its operation more robust.

## Claims

1. A reaction system for combustion of a combustible mixture of fuel and an oxygen-containing gas wherein a flowing stream of the combustible mixture, in vapor or gaseous form, is initially subject to partial combustion in the presence of a catalyst followed by complete combustion under non-catalytic conditions in a homogeneous combustion zone downstream from the catalyst comprising:
(a) a catalyst structure made up of a heat resistant support material composed of a plurality of common walls which form a multitude of adjacently disposed longitudinal channels for passage of the combustible mixture, wherein at least a part of the interior surface of a portion of the channels is coated with a catalyst for the combustible mixture and the interior surface of the remaining channels is not coated with catalyst such that the interior surface of the catalyst-coated channels are in heat exchange relationship with the interior surface of adjacent catalyst-free channels, and wherein the catalyst-coated channels have a configuration which forms a more tortuous flow passage for the reaction mixture than the flow passage formed by the catalyst-free channels, such that only a portion of the combustible mixture undergoes combustion to afford a partially-combusted, gaseous mixture flowing at elevated temperature from the outlet end of the catalyst structure;
(b) a homogeneous combustion zone comprising an enclosed space in fluid communication with the catalyst structure and located immediately downstream from the outlet end of the catalyst structure; and
(c) a means for inducing recirculation into the partially-combusted mixture flowing through the homogeneous combustion zone whereby homogeneous combustion of the partially-combusted mixture is stabilized within the region of recirculation and complete combustion of the partially-combusted mixture is promoted within the homogeneous combustion zone.

2. The reaction system of Claim 1, wherein the catalyst-coated channels of the catalyst structure are periodically altered through a change in cross-sectional area, a change in direction along the longitudinal axis of the channels or a combination of both changes in cross-sectional area and direction along their longitudinal axis such that the flow direction of at least a portion of the gaseous reaction mixture in the catalyst-coated channels is changed at least a plurality of points as the gaseous reaction mixture passes through the catalyst-coated channels while the catalyst-free channels are substantially straight and of unaltered cross-sectional area along their longitudinal axis, such that the flow direction of gaseous reaction mixture through the catalyst-free channels is substantially unaltered.

3. The reaction system of Claim 2, wherein the catalyst-coated channels are varied in cross-sectional area through a repeated inward and outward bending of the channel walls along the longitudinal axis of the channels or through the use of flaps, baffles or other obstructions placed at a plurality of points along the longitudinal axis of the channels to partially obstruct the gaseous reaction mixture flow direction.

4. The reaction system of Claim 3, wherein the catalyst-coated channels are varied in the cross-sectional area by the repeated inward and outward bending of the walls of the catalyst-coated channels which is accomplished with catalyst-coated channels which are corrugated in a herringbone pattern using corrugated sheets stacked in a non-nesting fashion.

5. The reaction system of Claim 4, wherein the catalyst-coated channels and the catalyst-free channels are formed by a repeating three layer structure comprised of a first layer of corrugated sheet with longitudinal peaks separated by flat regions stacked upon a second layer composed of corrugated sheet in which the corrugations are formed as adjacent longitudinal ridges and valleys with these ridges and valleys forming a herringbone pattern along the length of the sheet making up the second layer with the second layer being stacked in non-nesting fashion upon a third layer composed of corrugated metallic sheet in which the corrugations are formed as adjacent longitudinal ridges and valleys with the ridges and valleys forming a herringbone pattern along the length of the sheet making up the third layer, and with catalyst for the reaction mixture being coated on the bottom side of the first layer and top side of the third layer such that catalyst-free channels are formed when the first layer of the repeating structure is set under the third layer of the next adjacent repeating three layer structure in a stacked pattern and catalyst-coated channels are formed between the bottom of the first layer and the top of the second layer and between the bottom of the second layer and the top of the third layer of the repeating three layer structure.

6. The reaction system of claim 1, wherein:
(i) the catalyst-coated channels have a smaller average hydraulic diameter (Dₕ) than the catalyst-free channels; and
(ii) the catalyst-coated channels have a higher film heat transfer coefficient (h) than the catalyst-free channels.

7. The reaction system of claim 6, wherein the catalyst-coated channels have a film heat transfer coefficient (h) which is more than 1.5 times greater than the h for catalyst-free channels and the catalyst-coated channels represent from about 20% to about 80% of the total open frontal area in the catalyst structure.

8. A reaction system for combustion of a combustible mixture of fuel and an oxygen-containing gas wherein a flowing stream of the combustible mixture, in vapor or gaseous form, is initially subject to partial combustion in the presence of a catalyst followed by complete combustion under non-catalytic conditions in a homogeneous combustion zone downstream from the catalyst comprising:
(a) a catalyst structure made up of a heat resistant support material composed of a plurality of common walls which form a multitude of adjacently disposed longitudinal channels for passage of the combustible mixture, wherein at least a part of the interior surface of a portion of the channels is coated with a catalyst for the combustible mixture and the interior surface of the remaining channels is not coated with catalyst such that the interior surface of the catalyst-coated channels are in heat exchange relationship with the interior surface of adjacent catalyst-free channels and wherein catalyst-coated channels have a lower average hydraulic diameter Dₕ than the catalyst-free channels and the numeric ratio of average Dₕ for the catalyst-coated channels divided by the average Dₕ for the catalyst-free channels is smaller than the numeric ratio of open frontal area of the catalyst-coated channels divided by the open frontal area of the catalyst-free channels, such that only a portion of the combustible mixture undergoes combustion to afford a partially-combusted, gaseous mixture flowing at elevated temperature from the outlet end of the catalyst structure;
(b) a homogeneous combustion zone comprising an enclosed space in fluid communication with the catalyst structure and located immediately downstream from the outlet end of the catalyst structure; and
(c) a means for inducing recirculation into the partially-combusted mixture flowing through the homogeneous combustion zone whereby complete combustion of the partially-combusted mixture is stabilized within the region of recirculation and complete combustion of the partially-combusted mixture is promoted within the homogeneous combustion zone.

9. The reaction system of claim 8, wherein the catalyst-coated channels have a higher film heat transfer coefficient (h) than the catalyst-free channels.

10. The reaction system of any one of Claims 1 to 9, wherein the means for inducing recirculation into the partially-combusted mixture flow is a flameholder positioned downstream from the outlet end of the catalyst structure.

11. The reaction system of Claim 10, wherein the flameholder is selected from a bluff body, a V-gutter, a cone, a perforated plate, a swirler or a means for changing the cross-sectional area of the homogeneous combustion zone in the direction of partially-combusted gas flow or any combination of these.

12. The reaction system of Claim 11, wherein the flameholder is positioned from about 0.2 to about 20 cm downstream from the outlet end of the catalyst structure.

13. The reaction system of Claim 12, wherein the flameholder provides a geometric flow blockage in the homogeneous combustion zone of from about 10 to about 70 percent.

14. The reaction system of Claim 12, wherein between about 10 to about 70 percent of the fuel in the combustible mixture is combusted in the catalyst structure.

15. The reaction system of Claim 12, wherein between about 20 to about 70 percent of the fuel in the combustible mixture is combusted in the catalyst structure.

16. The reaction system of Claims 14 or 15, wherein the temperature of the partially-combusted, gaseous mixture flowing out of the outlet end of the catalyst structure is between about 700 and 1000°C.

17. A process for the combustion of a combustible mixture comprising the steps of:
(a) mixing a fuel and an oxygen-containing gas to form a combustible mixture;
(b) contacting the mixture with a heat resistant catalyst support composed of a plurality of common walls which form a multitude of adjacently disposed longitudinal channels for passage of the combustible mixture wherein at least a part of the interior surface of a portion of the channels is coated with a catalyst for the combustible mixture and the interior surface of the remaining channels is not coated with catalyst such that the interior surface of the catalyst-coated channels are in heat exchange relationship with the interior surface of adjacent catalyst-free channels, and wherein the catalyst-coated channels have a higher film heat transfer coefficient (h) than the catalyst-free channels, the catalyst-coated channels have a smaller average hydraulic diameter Dₕ than the catalyst-free channels, and the catalyst-coated channels form a more tortuous flow passage for the combustible mixture than the flow passage formed by the catalyst-free channels, thereby combusting a portion of the combustible mixture to afford a partially-combusted, gaseous mixture; and
(c) passing the partially-combusted, gaseous mixture to a homogeneous combustion zone equipped with a flameholder to effect recirculation of at least a portion of the partially-combusted mixture such that homogeneous combustion is stabilized within the region of recirculation and essentially complete combustion of the partially-combusted mixture is obtained.

18. A process for the combustion of a combustible mixture comprising the steps of:
(a) mixing a fuel and an oxygen-containing gas to form a combustible mixture;
(b) contacting the mixture with a heat resistant catalyst support composed of a plurality of common walls which form a multitude of adjacently disposed longitudinal channels for passage of the combustible mixture wherein at least a part of the interior surface of a portion of the channels is coated with a catalyst for the combustible mixture and the interior surface of the remaining channels is not coated with catalyst such that the interior surface of the catalyst-coated channels are in heat exchange relationship with the interior surface of adjacent catalyst-free channels, and wherein the catalyst-coated channels have a higher film heat transfer coefficient (h) than the catalyst-free channels, the catalyst-coated channels have a smaller average hydraulic diameter Dₕ than the catalyst-free channels, and the numeric ratio of average Dₕ for the catalyst-coated channels divided by the average Dₕ for the catalyst-free channels is smaller than the numeric ratio of open frontal area of the catalyst-coated channels divided by the open frontal area of the catalyst-free channels, thereby combusting a portion of the combustible mixture to afford a partially-combusted, gaseous mixture; and
(c) passing the partially-combusted, gaseous mixture to a homogeneous combustion zone equipped with a flameholder to effect recirculation of at least a portion of the partially-combusted mixture such that homogeneous combustion is stabilized within the region of recirculation and essentially complete combustion of the partially-combusted mixture is obtained.

19. The process of Claims 17 or 18, wherein the heat transfer surface area between the catalyst-coated channels and the catalyst-free channels divided by the total channel volume in the structure is greater than about 0.5 mm⁻¹.

20. The process of Claims 17 or 18, wherein the flameholder is selected from a bluff body, a V-gutter, a cone, a perforated plate, a swirler or a means for changing the cross-sectional area of the homogeneous combustion zone in the direction of partially-combusted gas flow or any combustion of these.

21. The process of Claim 20, wherein the flameholder is positioned from about 0.2 to about 20 cm downstream from the outlet end of the catalyst structure.

22. The process of Claim 21, wherein the flameholder provides a geometric flow blockage in the homogeneous combustion zone of from about 10 to about 70 percent.

23. The process of Claim 22, wherein between about 10 to about 70 percent of the fuel in the combustible mixture is combusted in the catalyst structure.

24. The process of Claim 23, wherein the temperature of the partially-combusted, gaseous mixture flowing out of the outlet end of the catalyst structure is between about 700 and 1000°C.

## Patentansprüche

1. Reaktionssystem für die Verbrennung einer brennbaren Mischung aus Brennstoff und einem sauerstoffhaltigen Gas, wobei ein in Dampf- bzw. Gasform vorhandener Fließstrom der brennbaren Mischung zunächst bei Vorhandensein eines Katalysators einer Teilverbrennung unterzogen wird und anschließend eine vollständige Verbrennung unter nichtkatalytischen Bedingungen in einem dem Katalysator nachgeschalteten homogenen Verbrennungsbereich erfolgt, welches umfasst:
(a) eine aus einem wärmebeständigen Hilfsmittel bestehende, sich aus einer Vielzahl von gemeinsamen Wänden, die eine Mehrzahl von angrenzenden Längskanälen zur Durchleitung der brennbaren Mischung bilden, zusammensetzende Katalysatorstruktur, wobei zumindest ein Teil der Innenfläche eines Teils der Kanäle mit einem Katalysator für die brennbare Mischung beschichtet wird und die Innenfläche der verbleibenden Kanäle nicht mit einem Katalysator beschichtet wird, so dass die Innenfläche der mit dem Katalysator beschichteten Kanäle in wärmeübertragender Beziehung zu der Innenfläche benachbarter katalysatorfreien Kanäle steht, und wobei die mit dem Katalysator beschichteten Kanäle ausgelegt sind, dass sie derart für die Reakationsmischung eine gekrümmtere Stromdurchführung als die durch die katalysatorfreien Kanäle gebildeten Stromdurchführung aufweisen, so dass nur ein Teil der brennbaren Mischung zum Ermöglichen einer teilverbrannten, gasförmigen Mischung, die bei erhöhter Temperatur aus dem Auslassende der Katalysatorstruktur strömt, einer Verbrennung unterzogen wird;
(b) einen homogenen Verbrennungsbereich, der einen in Fluidverbindung mit der Katalysatorstruktur stehenden geschlossenen Raum umfasst und der direkt stromabwärts von dem Auslassende der Katalysatorstruktur angeordnet ist; und
(c) Mittel zur Einleitung einer Rückführung in die teilverbrannte durch den homogenen Verbrennungsbereich strömende Mischung, wobei die homogene Verbrennung der teilverbrannten Mischung innerhalb des Rückführungsbereichs stabilisiert wird und eine vollständige Verbrennung der teilverbrannten Mischung innerhalb des homogenen Verbrennungsbereichs gefördert wird.

2. Reaktionssystem nach Anspruch 1, **dadurch gekennzeichnet, dass** die mit dem Katalysator beschichteten Kanäle der Katalysatorstruktur periodisch derart über eine Änderung der Querschnittsfläche, eine Richtungsänderung entlang der Längsachse der Kanäle oder eine Kombination der beiden Änderungen der Querschnittsfläche und der Richtung entlang der jeweiligen Längsachse, dass bei Strömen der gasförmigen Mischung durch die mit dem Katalysator beschichteten Kanäle die Strömungsrichtung mindestens eines Teils der gasförmigen Reaktionsmischung in den mit dem Katalysator beschichteten Kanälen zumindest an einer Vielzahl an Stellen derart verändert wird, während die katalysatorfreien Kanäle entlang ihrer jeweiligen Längsachse im Wesentlichen gerade sind und eine unveränderte Querschnittsfläche aufweisen, dass die Strömungsrichtung der gasförmigen Reaktionsmischung durch die katalysatorfreien Kanäle im Wesentlichen unverändert bleibt.

3. Reaktionssystem nach Anspruch 2, **dadurch gekennzeichnet, dass** die mit dem Katalysator beschichteten Kanäle über eine wiederholte nach innen bzw. außen gerichtete Krümmung der Kanalwandungen entlang der Längsachse der Kanäle bzw. über die Verwendung von Klappen bzw. Prallflächen oder sonstige an einer Vielzahl an Stellen entlang der Längsachse der Kanäle angebrachte Hindernisse zur teilweisen Behinderung der Strömungsrichtung der gasförmigen Reaktionsmischung in der Querschnittsfläche geändert werden.

4. Reaktionssystem nach Anspruch 3, **dadurch gekennzeichnet, dass** die mit dem Katalysator beschichteten Kanäle über die wiederholte nach innen bzw. außen gerichtete Krümmung der Wandungen der mit dem Katalysator beschichteten Kanäle in der Querschnittsfläche geändert werden, was mittels mit dem Katalysator beschichteten Kanäle erfolgt, die unter Verwendung von nicht ineinander greifend gestapelten im Fischgrätmuster gewellten Wellblechen gewellt werden.

5. Reaktionssystem nach Anspruch 4, **dadurch gekennzeichnet, dass** die mit dem Katalysator beschichteten Kanäle und die katalysatorfreien Kanäle durch eine sich wiederholende dreilagige Struktur gebildet werden, die aus Folgendem besteht: einer ersten Lage aus Wellblech mit durch ebene Bereiche getrennten Längshöhen, die auf einer zweiten Lage gestapelt wird, die aus Wellblech besteht, in dem die Wellen als benachbarte Längserhebungen bzw. -täler gebildet sind, wobei diese Erhebungen und Täler ein Fischgrätmuster entlang der Länge des die zweite Lage ausbildenden Blechs bilden, wobei die zweite Lage in nicht ineinandergreifender Weise auf einer dritten Lage gestapelt wird, die aus Wellblech besteht, in dem die Wellen als benachbarte Längserhebungen bzw. -täler gebildet sind, wobei die Erhebungen und Täler ein Fischgrätmuster entlang der Länge des die dritte Lage ausbildenden Blechs bilden, und wobei der Katalysator für die Reaktionsmischung derart auf die Unterseite der ersten Lagen und die Oberseite der dritten Lage aufgetragen wird, dass bei stapelförmiger Einlagerung der ersten Lage der sich wiederholenden Struktur unter die dritte Lage der nächstanliegenden sich wiederholenden dreilagigen Struktur katalysatorfreie Kanäle gebildet werden, und mit dem Katalysator beschichtete Kanäle zwischen der Unterseite der ersten Lage und der Oberseite der zweiten Lage und zwischen der Unterseite der zweiten Lage und der Oberseite der dritten Lage der sich wiederholenden dreilagigen Struktur gebildet werden.

6. Reaktionssystem nach Anspruch 1, **dadurch gekennzeichnet, dass**
(i) die mit dem Katalysator beschichteten Kanäle einen kleineren durchschnittlichen hydraulischen Durchmesser (Dₕ) als die katalysatorfreien Kanäle aufweisen; und
(ii) die mit dem Katalysator beschichteten Kanäle einen höheren Folienwärmeübergangskoeffizienten (h) als die katalysatorenfreien Kanäle aufweisen.

7. Reaktionssystem nach Anspruch 6, **dadurch gekennzeichnet, dass** die mit dem Katalysator beschichteten Kanäle einen Folienwärmeübergangskoeffizienten (h) aufweisen, der mehr als 1,5 Mal höher als der h-Wert für die katalysatorfreien Kanäle ist, und die mit dem Katalysator beschichteten Kanäle etwa 20 % bis etwa 80 % des gesamten offenen Vorderbereichs in der Katalysatorstruktur ausmachen.

8. Reaktionssystem für die Verbrennung einer brennbaren Mischung aus Brennstoff und einem sauerstoffhaltigen Gas, wobei ein in Dampf- bzw. Gasform vorhandener Fließstrom der brennbaren Mischung zunächst bei Vorhandensein eines Katalysators einer Teilverbrennung unterzogen wird und anschließend eine vollständige Verbrennung unter nichtkatalytischen Bedingungen in einem dem Katalysator nachgeschalteten homogenen Verbrennungsbereich erfolgt, welches umfasst:
(a) eine aus einem wärmebeständigen Hilfsmittel bestehende, sich aus einer Vielzahl von gemeinsamen Wänden, die eine Mehrzahl von angrenzenden Längskanälen zur Durchleitung der brennbaren Mischung bilden, zusammensetzende Katalysatorstruktur, wobei zumindest ein Teil der Innenfläche eines Teils der Kanäle mit einem Katalysator für die brennbare Mischung beschichtet wird und die Innenfläche der verbleibenden Kanäle nicht mit einem Katalysator beschichtet wird, so dass die Innenfläche der mit dem Katalysator beschichteten Kanäle in wärmeübertragender Beziehung zu der Innenfläche benachbarter katalysatorfreien Kanäle steht, und wobei die mit dem Katalysator beschichteten Kanäle einen niedrigeren durchschnittlichen hydraulischen Durchmesser Dₕ als die katalysatorfreien Kanäle aufweisen und das numerische Verhältnis des durch den durchschnittlichen Dₕ-Wert für die katalysatorfreien Kanäle geteilten durchschnittlichen Dₕ-Werts für die mit dem Katalysator beschichteten Kanäle kleiner als das numerische Verhältnis des offenen Vorderbereichs der mit dem Katalysator beschichteten Kanäle geteilt durch den offenen Vorderbereich der katalysatorfreien Kanäle ist, so dass nur ein Teil der brennbaren Mischung zum Ermöglichen einer teilverbrannten, gasförmigen Mischung, die bei erhöhter Temperatur aus dem Auslassende der Katalysatorstruktur strömt, einer Verbrennung unterzogen wird;
(b) einen homogenen Verbrennungsbereich, der einen in Fluidverbindung mit der Katalysatorstruktur stehenden geschlossenen Raum umfasst und der direkt stromabwärts von dem Auslassende der Katalysatorstruktur angeordnet ist; und
(c) Mittel zur Einleitung einer Rückführung in die teilverbrannte durch den homogenen Verbrennungsbereich strömende Mischung, wobei die vollständige Verbrennung der teilverbrannten Mischung innerhalb des Rückführungsbereichs stabilisiert wird und eine vollständige Verbrennung der teilverbrannten Mischung innerhalb des homogenen Verbrennungsbereichs gefördert wird.

9. Reaktionssystem nach Anspruch 8, **dadurch gekennzeichnet, dass** die mit dem Katalysator beschichteten Kanäle einen höheren Folienwärmübergangskoeffizienten (h) als die katalysatorfreien Kanäle aufweisen.

10. Reaktionssystem nach einem der Ansprüche 1 bis 9, **dadurch gekennzeichnet, dass** das Mittel zur Einleitung der Rückführung in den teilverbrannten Mischungsstrom ein stromabwärts von dem Auslassende der Katalysatorstruktur angeordneter Flammenstabilisator ist.

11. Reaktionssystem nach Anspruch 10, **dadurch gekennzeichnet, dass** der Flammenstabilisator aus einem Körper mit hohem Strömungswiderstand, einer V-Rinne, einem Konus, einer gelochten Platte, einem Drallkörper oder aus einem Mittel zur Veränderung der Querschnittsfläche des homogenen Verbrennungsbereichs in Richtung der teilverbrannten Gasströmung bzw. einer beliebigen Kombination daraus gewählt wird.

12. Reaktionssystem nach Anspruch 11, **dadurch gekennzeichnet, dass** der Flammenstabilisator etwa 0,2 bis etwa 20 cm stromabwärts von dem Auslassende der Katalysatorstruktur angeordnet ist.

13. Reaktionssystem nach Anspruch 12, **dadurch gekennzeichnet, dass** der Flammenstabilisator eine geometrische Strömungssperre im homogenen Verbrennungsbereich etwa. 10 bis etwa 70 Prozent darstellt.

14. Reaktionssystem nach Anspruch 12, **dadurch gekennzeichnet, dass** etwa 10 bis etwa 70 Prozent des in der brennbaren Mischung vorhandenen Brennstoffs in der Katalysatorstruktur verbrannt wird.

15. Reaktionssystem nach Anspruch 12, **dadurch gekennzeichnet, dass** etwa 20 bis etwa 70 Prozent des in der brennbaren Mischung vorhandenen Brennstoffs in der Katalysatorstruktur verbrannt wird.

16. Reaktionssystem nach Anspruch 14 oder 15, **dadurch gekennzeichnet, dass** die Temperatur der aus dem Auslassende der Katalysatorstruktur strömenden, teilverbrannten gasförmigen Mischung bei etwa 700 bis 1000°C liegt.

17. Verfahren zur Verbrennung einer brennbaren Mischung, welches die Schritte umfasst:
(a) Mischung eines Brennstoffs und eines sauerstoffhaltigen Gases zur Bildung einer brennbaren Mischung;
(b) Kontaktierung der Mischung mit einem wärmebeständigen katalytischen Hilfsmittel, das aus einer Vielzahl von gemeinsamen Wandungen besteht, die eine Mehrzahl von angrenzenden Längskanälen zur Durchleitung der brennbaren Mischung bilden, wobei zumindest ein Teil der Innenfläche eines Teils der Kanäle mit einem Katalysator für die brennbare Mischung beschichtet wird und die Innenfläche der verbleibenden Kanäle nicht mit einem Katalysator beschichtet wird, so dass die Innenfläche der mit dem Katalysator beschichteten Kanäle in wärmeübertragender Beziehung zu der Innenfläche benachbarter katalysatorfreien Kanäle steht, und wobei die mit dem Katalysator beschichteten Kanäle einen höheren Folienwärmeübergangskoeffizienten (h) als die katalysatorfreien Kanäle aufweisen, die mit dem Katalysator beschichteten Kanäle einen niedrigeren durchschnittlichen hydraulischen Durchmesser Dₕ als die katalysatorfreien Kanäle aufweisen und die mit dem Katalysator beschichteten Kanäle eine gekrümmtere Stromdurchführung für die brennbare Mischung als die durch die katalysatorfreien Kanäle gebildete Stromdurchführung bilden, wodurch ein Teil der brennbaren Mischung zum Ermöglichen einer teilverbrannten, gasförmigen Mischung verbrannt wird; und
(c) Weiterleiten der teilverbrannten, gasförmigen Mischung an einen mit einem Flammenstabilisator zur Bewirkung der Rückführung mindestens eines Teils der teilverbrannten Mischung ausgestatten homogenen Verbrennungsbereich, so dass die homogene Verbrennung innerhalb des Rückführungsbereichs stabilisiert wird und eine im Wesentlichen vollständige Verbrennung der teilverbrannten Mischung erhalten wird.

18. Verfahren zur Verbrennung einer brennbaren Mischung, welches die Schritte umfasst:
(a) Mischung eines Brennstoffs und eines sauerstoffhaltigen Gases zur Bildung einer brennbaren Mischung;
(b) Kontaktierung der Mischung mit einem wärmebeständigen katalytischen Hilfsmittel, das aus einer Vielzahl von gemeinsamen Wandungen besteht, die eine Mehrzahl von angrenzenden Längskanälen zur Durchleitung der brennbaren Mischung bilden, wobei zumindest ein Teil der Innenfläche eines Teils der Kanäle mit einem Katalysator für die brennbare Mischung beschichtet wird und die Innenfläche der verbleibenden Kanäle nicht mit einem Katalysator beschichtet wird, so dass die Innenfläche der mit dem Katalysator beschichteten Kanäle in wärmeübertragender Beziehung zu der Innenfläche benachbarter katalysatorfreien Kanäle steht, und wobei die mit dem Katalysator beschichteten Kanäle einen höheren Folienwärmeübergangskoeffizienten (h) als die katalysatorfreien Kanäle aufweisen, die mit dem Katalysator beschichteten Kanäle einen niedrigeren durchschnittlichen hydraulischen Durchmesser Dₕ als die katalysatorfreien Kanäle aufweisen und das numerische Verhältnis des durch den durchschnittlichen Dₕ-Wert für die katalysatorfreien Kanäle geteilten durchschnittlichen Dₕ-Werts für die mit dem Katalysator beschichteten Kanäle kleiner als das numerische Verhältnis des offenen Vorderbereichs der mit dem Katalysator beschichteten Kanäle geteilt duch die offene Vorderfläche der katalysatorfreien Kanäle ist, wodurch ein Teil der brennbaren Mischung zum Ermöglichen einer teilverbrannten, gasförmigen Mischung verbrannt wird; und
(c) Weiterleiten der teilverbrannten, gasförmigen Mischung an einen mit einem Flammenstabilisator zur Bewirkung der Rückführung mindestens eines Teils der teilverbrannten Mischung ausgestatten homogenen Verbrennungsbereich, so dass die homogene Verbrennung innerhalb des Rückführungsbereichs stabilisiert wird und eine im Wesentlichen vollständige Verbrennung der teilverbrannten Mischung erhalten wird.

19. Verfahren nach Anspruch 17 oder 18, **dadurch gekennzeichnet, dass** die durch das gesamte in der Struktur vorhandene Kanalvolumen geteilte Wärmeübertragungsfläche zwischen den mit dem Katalysator beschichteten Kanälen und den katalysatorfreien Kanälen größer als ca. 0,5 mm⁻¹ ist.

20. Verfahren nach Anspruch 17 oder 18, **dadurch gekennzeichnet, dass** der Flammenstabilisator aus einem Körper mit hohem Strömungswiderstand, einer V-Rinne, einem Konus, einer gelochten Platte, einem Drallkörper oder aus einem Mittel zur Veränderung der Querschnittsfläche des homogenen Verbrennungsbereichs in Richtung der teilverbrannten Gasströmung bzw. einer beliebigen Kombination daraus gewählt wird.

21. Verfahren nach Anspruch 20, **dadurch gekennzeichnet, dass** der Flammenstabilisator etwa 0,2 bis etwa 20 cm stromabwärts von dem Auslassende der Katalysatorstruktur angeordnet ist.

22. Verfahren nach Anspruch 21, **dadurch gekennzeichnet, dass** der Flammenstabilisator eine geometrische Strömungssperre im homogenen Verbrennungsbereich von etwa 10 bis etwa 70 Prozent darstellt.

23. Verfahren nach Anspruch 22, **dadurch gekennzeichnet, dass** etwa 10 bis etwa 70 Prozent des in der brennbaren Mischung vorhandenen Brennstoffs in der Katalysatorstruktur verbrannt wird.

24. Verfahren nach Anspruch 23, **dadurch gekennzeichnet, dass** die Temperatur der aus dem Auslassende der Katalysatorstruktur strömenden, teilverbrannten gasförmigen Mischung bei etwa 700 bis 1000°C liegt.

## Revendications

1. Système de réaction pour combustion d'un mélange combustible de carburant et d'un gaz contenant de l'oxygène, dans lequel un flux d'écoulement du mélange combustible, sous forme de vapeur ou de gaz, est soumis initialement à une combustion partielle en présence d'un catalyseur, suivie par une combustion complète dans des conditions non-catalytiques dans une zone de combustion homogène située en aval du catalyseur, comportant :
(a) une structure de catalyseur réalisée en un matériau de support résistant à la chaleur, constituée d'une pluralité de parois communes qui forment une multitude de canaux longitudinaux disposés de manière adjacente pour le passage du mélange combustible, dans laquelle au moins une partie de la surface intérieure d'une partie des canaux est revêtue de catalyseur pour le mélange combustible, et la surface intérieure des canaux restants n'est pas revêtue de catalyseur, de telle sorte que la surface intérieure des canaux revêtus de catalyseur est dans une relation d'échange thermique avec la surface intérieure des canaux sans catalyseur adjacents, et dans laquelle les canaux revêtus de catalyseur ont une configuration qui forme un passage d'écoulement plus tortueux pour le mélange réactionnel que le passage d'écoulement formé par les canaux sans catalyseur, de telle sorte que seule une partie du mélange combustible subit une combustion pour permettre à un mélange gazeux partiellement brûlé de s'écouler à température élevée à partir de l'extrémité de sortie de la structure de catalyseur,
(b) une zone de combustion homogène comportant un espace clos en communication de fluide avec la structure de catalyseur, et positionnée immédiatement en aval de l'extrémité de sortie de la structure de catalyseur, et
(c) des moyens pour provoquer une remise en circulation dans le mélange partiellement brûlé s'écoulant à travers la zone de combustion homogène, de sorte qu'une combustion homogène du mélange partiellement brûlé est stabilisée dans la zone de remise en circulation, et une combustion complète du mélange partiellement brûlé est favorisée dans la zone de combustion homogène.

2. Système de réaction selon la revendication 1, dans lequel les canaux revêtus de catalyseur de la structure de catalyseur sont modifiés périodiquement par l'intermédiaire d'un changement de surface en coupe, d'un changement de direction le long de l'axe longitudinal des canaux, ou d'une combinaison des deux changements de surface en coupe et de direction le long de leur axe longitudinal, de telle sorte que la direction d'écoulement d'au moins une partie du mélange réactionnel gazeux dans les canaux revêtus d'un catalyseur est modifiée au moins partiellement au niveau d'une pluralité de points lorsque le mélange réactionnel gazeux passe à travers les canaux revêtus de catalyseur, tandis que les canaux sans catalyseur sont pratiquement rectilignes et ont une surface en coupe non modifiée le long de leur axe longitudinal, de telle sorte que la direction d'écoulement du mélange réactionnel gazeux à travers les canaux sans catalyseur est pratiquement inchangée.

3. Système de réaction selon la revendication 2, dans lequel les canaux revêtus de catalyseur ont une surface en coupe modifiée par l'intermédiaire d'une incurvation répétée vers l'intérieur et vers l'extérieur des parois de canaux le long de l'axe longitudinal des canaux, ou par l'intermédiaire de l'utilisation de volets, de déflecteurs ou d'autres obstacles positionnés au niveau d'une pluralité de points le long de l'axe longitudinal des canaux, pour obstruer partiellement la direction d'écoulement de mélange réactionnel gazeux.

4. Système de réaction selon la revendication 3, dans lequel les canaux revêtus de catalyseur ont une surface en coupe modifiée par l'intermédiaire de l'incurvation répétée vers l'intérieur et vers l'extérieur des parois des canaux revêtus de catalyseur, qui est accomplie à l'aide de canaux revêtus d'un catalyseur qui sont ondulés selon un motif de chevrons en utilisant des feuilles ondulées empilées d'une manière sans emboîtement.

5. Système de réaction selon la revendication 4, dans lequel les canaux revêtus de catalyseur et les canaux sans catalyseur sont formés par l'intermédiaire d'une structure à trois couches se répétant, constituée d'une première couche en feuille ondulée munie de pics longitudinaux séparés par des zones plates, empilées, sur une deuxième couche constituée de feuille ondulée dans laquelle les ondulations ont la forme de crêtes et de vallées longitudinales adjacentes, ces crêtes et vallées formant un motif en chevrons le long de la longueur de la feuille constituant la deuxième couche, la deuxième couche étant empilée d'une manière sans emboîtement sur une troisième couche constituée de feuille métallique ondulée dans laquelle les ondulations ont la forme de crêtes et de vallées longitudinales adjacentes, les crêtes et les vallées formant un motif en chevrons le long de la longueur de la feuille constituant la troisième couche, et le catalyseur pour le mélange réactionnel étant sous forme de revêtement sur le côté inférieur de la première couche et sur le côté supérieur de la troisième couche, de telle sorte que des canaux sans catalyseur sont formés lorsque la première couche de la structure se répétant est établie en dessous de la troisième couche de la structure à trois couches se répétant adjacente suivante selon un motif empilé, et des canaux revêtus de catalyseur sont formés entre la partie inférieure de la première couche et la partie supérieure de la deuxième couche, et entre la partie inférieure de la deuxième couche et la partie supérieure de la troisième couche de la structure à trois couches se répétant.

6. Système de réaction selon la revendication 1, dans lequel :
(i) les canaux revêtus de catalyseur ont un diamètre hydraulique moyen (Dₕ) plus petit que les canaux sans catalyseur, et
(ii) les canaux revêtus de catalyseur ont un coefficient de transfert thermique de film (h) plus élevé que les canaux sans catalyseur.

7. Système de réaction selon la revendication 6, dans lequel les canaux revêtus de catalyseur ont un coefficient de transfert thermique de film (h) qui est plus de 1,5 fois plus grand que le h des canaux sans catalyseur, et les canaux revêtus de catalyseur représentent d'environ 20 % à environ 80 % de la surface frontale ouverte totale de la structure de catalyseur.

8. Système de réaction pour combustion d'un mélange combustible de carburant et d'un gaz contenant de l'oxygène, dans lequel un flux d'écoulement du mélange combustible, sous forme de vapeur ou de gaz, est soumis initialement à une combustion partielle en présence d'un catalyseur, suivie par une combustion complète dans des conditions non-catalytiques dans une zone de combustion homogène située en aval du catalyseur, comportant :
(a) une structure de catalyseur réalisée en matériau de support résistant à la chaleur, constituée d'une pluralité de parois communes qui forment une multitude de canaux longitudinaux disposés de manière adjacente pour le passage du mélange combustible, dans laquelle au moins une partie de la surface intérieure d'une partie des canaux est revêtue de catalyseur pour le mélange combustible, et la surface intérieure des canaux restants n'est pas revêtue de catalyseur, de telle sorte que la surface intérieure des canaux revêtus de catalyseur est dans une relation d'échange thermique avec la surface intérieure des canaux sans catalyseur adjacents, et dans laquelle les canaux revêtus d'un catalyseur ont un diamètre hydraulique moyen (Dₕ) plus petit que les canaux sans catalyseur, et le rapport numérique de Dₕ moyen des canaux revêtus de catalyseur divisé par le Dₕ moyen des canaux sans catalyseur est inférieur au rapport numérique de la surface frontale ouverte des canaux revêtus de catalyseur divisée par la surface frontale ouverte des canaux sans catalyseur, de telle sorte que seule une partie du mélange combustible subit une combustion pour permettre à un mélange gazeux partiellement brûlé de s'écouler à une température élevée à partir de l'extrémité de sortie de la structure de catalyseur,
(b) une zone de combustion homogène comportant un espace clos en communication de fluide avec la structure de catalyseur, et positionnée immédiatement en aval de l'extrémité de sortie de la structure de catalyseur, et
(c) des moyens pour provoquer une remise en circulation dans le mélange partiellement brûlé s'écoulant à travers la zone de combustion homogène, de sorte qu'une combustion complète du mélange partiellement brûlé est stabilisée dans la zone de remise en circulation, et une combustion complète du mélange partiellement brûlé est favorisée dans la zone de combustion homogène.

9. Système de réaction selon la revendication 8, dans lequel les canaux revêtus de catalyseur ont un coefficient de transfert thermique de film (h) plus élevé que les canaux sans catalyseur.

10. Système de réaction selon l'une quelconque des revendications 1 à 9, dans lequel les moyens pour provoquer une remise en circulation dans l'écoulement de mélange partiellement brûlé sont constitués d'un porte-flamme positionné en aval de l'extrémité de sortie de la structure de catalyseur.

11. Système de réaction selon la revendication10, dans lequel le porte-flamme est sélectionné parmi un corps non-profilé, une gouttière en forme de V, un cône, une plaque perforée, un dispositif de tourbillonnement ou des moyens pour modifier la surface en coupe de la zone de combustion homogène dans la direction d'écoulement de gaz partiellement brûlé, ou une combinaison quelconque de ceux-ci.

12. Système de réaction selon la revendication 11, dans lequel le porte-flamme est positionné entre environ 0,2 et environ 20 cm en aval de l'extrémité de sortie de la structure de catalyseur.

13. Système de réaction selon la revendication 12, dans lequel le porte-flamme fournit un blocage d'écoulement géométrique dans la zone de combustion homogène d'environ 10 à environ 70 %.

14. Système de réaction selon la revendication 12, dans lequel entre environ 10 et environ 70 % du carburant du mélange combustible est brûlé dans la structure de catalyseur.

15. Système de réaction selon la revendication 12, dans lequel entre environ 20 et environ 70 % du carburant du mélange de combustible est brûlé dans la structure de catalyseur.

16. Système de réaction selon la revendication 14 ou 15, dans lequel la température du mélange gazeux partiellement brûlé s'écoulant vers l'extérieur de l'extrémité de sortie de la structure de catalyseur est comprise entre environ 700 et 1000°C.

17. Procédé pour la combustion d'un mélange combustible comportant les étapes consistant à :
(a) mélanger un carburant et un gaz contenant de l'oxygène pour former un mélange combustible,
(b) mettre en contact le mélange avec un support de catalyseur résistant à la chaleur constitué d'une pluralité de parois communes qui forment une multitude de canaux longitudinaux disposés de manière adjacente pour le passage du mélange combustible, dans lesquels au moins une partie de la surface intérieure d'une partie des canaux est revêtue d'un catalyseur pour le mélange combustible, et la surface intérieure des canaux restants n'est pas revêtue de catalyseur, de telle sorte que la surface intérieure des canaux revêtus de catalyseur est dans une relation d'échange thermique avec la surface intérieure de canaux sans catalyseur adjacents, et dans lesquels les canaux revêtus de catalyseur ont un coefficient de transfert de chaleur de film (h) plus élevé que les canaux sans catalyseur, les canaux revêtus de catalyseur ont un diamètre hydraulique moyen Dₕ plus petit que les canaux sans catalyseur, et les canaux revêtus de catalyseur forment un passage d'écoulement plus tortueux pour le mélange combustible que le passage d'écoulement formé par les canaux sans catalyseur, en brûlant ainsi une partie du mélange combustible pour donner un mélange gazeux partiellement brûlé, et
(c) faire passer le mélange gazeux partiellement brûlé vers une zone de combustion homogène munie d'un porte-flamme pour effectuer une remise en circulation d'au moins une partie du mélange partiellement brûlé, de telle sorte qu'une combustion homogène est stabilisée dans la zone de remise en circulation, et qu'une combustion sensiblement complète du mélange partiellement brûlé est obtenue.

18. Procédé pour la combustion d'un mélange combustible, comportant les étapes consistant à :
(a) mélanger un carburant et un gaz contenant de l'oxygène pour former un mélange combustible,
(b) mettre en contact le mélange avec un support de catalyseur résistant à la chaleur constitué d'une pluralité de parois communes qui forment une multitude de canaux longitudinaux disposés de manière adjacente pour le passage du mélange combustible, dans lesquels au moins une partie de la surface intérieure d'une partie des canaux est revêtue de catalyseur pour le mélange combustible, et la surface intérieure des canaux restants n'est pas revêtue de catalyseur, de telle sorte que la surface intérieure des canaux revêtus de catalyseur est dans une relation d'échange thermique avec la surface intérieure de canaux sans catalyseur adjacents, et dans lesquels les canaux revêtus de catalyseur ont un coefficient de transfert de chaleur de film (h) plus élevé que les canaux sans catalyseur, les canaux revêtus de catalyseur ont un diamètre hydraulique moyen Dₕ plus petit que les canaux sans catalyseur, et le rapport numérique de Dₕ moyen des canaux revêtus de catalyseur divisé par le Dₕ moyen des canaux sans catalyseur est inférieur au rapport numérique de la surface frontale ouverte des canaux revêtus de catalyseur divisée par la surface frontale ouverte des canaux sans catalyseur, de sorte qu'une partie du mélange combustible est brûlée pour donner un mélange gazeux partiellement brûlé, et
(c) faire passer le mélange gazeux partiellement brûlé vers une zone de combustion homogène munie d'un porte-flamme pour effectuer une remise en circulation d'au moins une partie du mélange partiellement brûlé, de telle sorte qu'une combustion homogène est partiellement stabilisée dans la zone de remise en circulation, et qu'une combustion pratiquement complète du mélange partiellement brûlé est obtenue.

19. Procédé selon la revendication 17 ou 18, dans lequel la surface superficielle de transfert thermique entre les canaux revêtus de catalyseur et les canaux sans catalyseur divisée par le volume de canal total dans la structure est supérieure à environ 0,5 mm⁻¹.

20. Procédé selon la revendication 17 ou 18, dans lequel le porte-flamme est sélectionné parmi un corps non-profilé, une gouttière en forme de V, un cône, une plaque perforée, un dispositif de tourbillonnement ou des moyens pour modifier la surface en coupe de la zone de combustion homogène dans la direction de l'écoulement de gaz partiellement brûlé, ou une combinaison quelconque de ceux-ci.

21. Procédé selon la revendication 20, dans lequel le porte-flamme est positionné entre environ 0,2 et environ 20 cm en aval de l'extrémité de sortie de la structure de catalyseur.

22. Procédé selon la revendication 21, dans lequel le support de flamme fournit un blocage d'écoulement géométrique dans la zone de combustion homogène d'environ 10 à environ 70 %.

23. Procédé selon la revendication 22, dans lequel entre environ 10 et environ 70 % du carburant du mélange combustible est brûlé dans la structure de catalyseur.

24. Procédé selon la revendication 23, dans lequel la température du mélange gazeux partiellement brûlé s'écoulant vers l'extérieur de l'extrémité de sortie de la structure de catalyseur est comprise entre environ 700 et 1000°C.
